



US011590547B2

(12) **United States Patent**  
Mizumura et al.

(10) **Patent No.:** US 11,590,547 B2  
(45) **Date of Patent:** Feb. 28, 2023

(54) **METHOD OF MANUFACTURING VARIABLE WALL THICKNESS STEEL PIPE AND VARIABLE WALL THICKNESS STEEL PIPE**

(71) **Applicant:** NIPPON STEEL & SUMITOMO METAL CORPORATION, Tokyo (JP)

(72) **Inventors:** Masaaki Mizumura, Tokyo (JP); Keinosuke Iguchi, Tokyo (JP); Hidehiro Arita, Tokyo (JP)

(73) **Assignee:** NIPPON STEEL CORPORATION, Tokyo (JP)

(\*) **Notice:** Subject to any disclaimer, the term of this patent is extended or adjusted under 35 U.S.C. 154(b) by 518 days.

(21) **Appl. No.:** 16/082,894

(22) **PCT Filed:** Feb. 14, 2017

(86) **PCT No.:** PCT/JP2017/005278

§ 371 (c)(1),

(2) **Date:** Sep. 6, 2018

(87) **PCT Pub. No.:** WO2017/154481

**PCT Pub. Date:** Sep. 14, 2017

(65) **Prior Publication Data**

US 2019/0076902 A1 Mar. 14, 2019

(30) **Foreign Application Priority Data**

Mar. 11, 2016 (JP) ..... JP2016-048657  
Dec. 19, 2016 (JP) ..... JP2016-245864

(51) **Int. Cl.**

B21C 37/16 (2006.01)  
B21D 39/20 (2006.01)

(Continued)

(52) **U.S. Cl.**

CPC ..... B21C 37/16 (2013.01); B21C 1/24 (2013.01); B21C 37/065 (2013.01); B21D 39/20 (2013.01); B21J 5/08 (2013.01); B21K 21/12 (2013.01)

(58) **Field of Classification Search**

CPC .. B21D 39/20; B21C 1/24; B21C 1/26; B21C 3/16; B21C 37/16; B21C 37/065; B21K 21/12; B21J 5/08

(Continued)

(56) **References Cited**

U.S. PATENT DOCUMENTS

1,511,091 A \* 10/1924 O'Rourke ..... B21C 3/16 72/467  
3,950,978 A \* 4/1976 Wassen ..... B21C 1/24 72/283

(Continued)

FOREIGN PATENT DOCUMENTS

CN 1528542 A 9/2004  
CN 1886210 A 12/2006

(Continued)

OTHER PUBLICATIONS

Technical Tidbits, "Strain Hardening & Strength", May 2010, Brush Wellman Inc., Issue 17 (Year: 2010).\*

(Continued)

*Primary Examiner* — Teresa M Ekiert

(74) **Attorney, Agent, or Firm:** Birch, Stewart, Kolasch & Birch, LLP

(57) **ABSTRACT**

There is provided a method of manufacturing a variable wall thickness steel pipe with a hollow tubular raw pipe. The method of manufacturing a variable wall thickness steel pipe includes locking the raw pipe in a die by thrusting a plug into the raw pipe from an one end side, so as to expand an outer shape on the one end side in a state, where the raw pipe is

(Continued)



disposed inside the die and movement of the raw pipe in a longitudinal direction is restricted; and performing ironing in which an inner shape of the raw pipe is expanded while the outer shape is maintained so that a thin portion is formed by further thrusting the plug toward the other end side of the raw pipe while the locked state of the raw pipe is maintained, whereas the restriction on the raw pipe is relaxed.

**12 Claims, 13 Drawing Sheets**

|              |      |         |                     |            |
|--------------|------|---------|---------------------|------------|
| 6,837,091    | B2 * | 1/2005  | Brochheuser .....   | B21C 1/18  |
|              |      |         |                     | 72/283     |
| 8,074,482    | B2 * | 12/2011 | Okui .....          | B21C 1/24  |
|              |      |         |                     | 72/283     |
| 8,210,017    | B2 * | 7/2012  | Suzuki .....        | B21C 51/00 |
|              |      |         |                     | 72/276     |
| 2007/0256467 | A1   | 11/2007 | Viegner, Jr. et al. |            |
| 2008/0115553 | A1   | 5/2008  | Brochheuser et al.  |            |
| 2009/0152065 | A1 * | 6/2009  | Shimai .....        | B21D 39/20 |
|              |      |         |                     | 188/379    |
| 2010/0139356 | A1   | 6/2010  | Brochheuser et al.  |            |

**FOREIGN PATENT DOCUMENTS**

|      |                   |           |
|------|-------------------|-----------|
| (51) | <b>Int. Cl.</b>   |           |
|      | <i>B21J 5/08</i>  | (2006.01) |
|      | <i>B21C 1/24</i>  | (2006.01) |
|      | <i>B21C 37/06</i> | (2006.01) |
|      | <i>B21K 21/12</i> | (2006.01) |

|      |                                       |                                                               |
|------|---------------------------------------|---------------------------------------------------------------|
| (58) | <b>Field of Classification Search</b> |                                                               |
|      | USPC .....                            | 72/276, 283, 370.01, 370.06, 370.1, 72/370.14, 370.23, 370.24 |

See application file for complete search history.

**(56) References Cited**

**U.S. PATENT DOCUMENTS**

|           |     |         |                |            |
|-----------|-----|---------|----------------|------------|
| 4,301,672 | A * | 11/1981 | Simon .....    | B21C 25/08 |
|           |     |         |                | 72/260     |
| 4,454,745 | A   | 6/1984  | Cudini         |            |
| 4,534,199 | A * | 8/1985  | Takaishi ..... | B21C 37/16 |
|           |     |         |                | 138/121    |
| 4,616,500 | A * | 10/1986 | Alexoff .....  | B21C 37/16 |
|           |     |         |                | 72/276     |
| 4,726,211 | A * | 2/1988  | Sunaga .....   | B21C 37/16 |
|           |     |         |                | 72/276     |
| 5,522,246 | A   | 6/1996  | Simon          |            |
| 5,533,376 | A * | 7/1996  | Wetzels .....  | B21C 1/24  |
|           |     |         |                | 72/283     |

|    |             |     |         |                  |
|----|-------------|-----|---------|------------------|
| CN | 101754820   | A   | 6/2010  |                  |
| CN | 102632093   | A   | 8/2012  |                  |
| EP | 0811444     | A1  | 12/1997 |                  |
| JP | 59047018    | A * | 3/1984  | ..... B21C 37/30 |
| JP | 59-73115    | A   | 4/1984  |                  |
| JP | 61123415    | A * | 6/1986  |                  |
| JP | 7-148516    | A   | 6/1995  |                  |
| JP | 9-327723    | A   | 12/1997 |                  |
| JP | 2001-121210 | A   | 5/2001  |                  |
| JP | 2006-110567 | A   | 4/2006  |                  |
| JP | 2006110567  | A * | 4/2006  |                  |
| JP | 2008-520440 | A   | 6/2008  |                  |
| JP | 2010-179319 | A   | 8/2010  |                  |
| JP | 2012-16712  | A   | 1/2012  |                  |

**OTHER PUBLICATIONS**

Chinese Office Action and Search Report for counterpart Chinese Application No. 201780016090.5, dated Jul. 2, 2019, with English translation of the Search Report only.  
 International Search Report for PCT/JP2017/005278 (PCT/ISA/210) dated May 23, 2017.  
 Written Opinion of the International Searching Authority for PCT/JP2017/005278 (PCT/ISA/237) dated May 23, 2017.  
 Extended European Search Report, dated Jan. 21, 2020, for corresponding European Application No. 17762824.5.

\* cited by examiner

- FIG. 1



**FIG. 2****FIG. 3**

**FIG. 4**

**FIG. 5****FIG. 6**

**FIG. 7**

FIG. 8



FIG. 9



**FIG. 10**

**FIG. 11****FIG. 12**

FIG. 13



**FIG. 14****FIG. 15**

**FIG. 16**

**FIG. 17****FIG. 18**

**FIG. 19****FIG. 20**

## 1

**METHOD OF MANUFACTURING VARIABLE  
WALL THICKNESS STEEL PIPE AND  
VARIABLE WALL THICKNESS STEEL PIPE**

TECHNICAL FIELD OF THE INVENTION

The present invention relates to a method of manufacturing a variable wall thickness steel pipe and a variable wall thickness steel pipe.

Priority is claimed on Japanese Patent Application No. 2016-048657, filed on Mar. 11, 2016 and Japanese Patent Application No. 2016-245864, filed on Dec. 19, 2016, the contents of which are incorporated herein by reference.

RELATED ART

It is desired that a vehicle body member constituting a vehicle body of an automobile has a part which absorbs collision energy by being crushed by impact load when an impact such as a collision is received, and a part which protects the vehicle body without being crushed. In order to provide such a vehicle body member, utilization of a variable wall thickness steel pipe having a thickness varying in a longitudinal direction has been studied.

For example, as a method of manufacturing a drawn steel pipe having a plurality of diameters, FIG. 7 of Patent Document 1 discloses a method of manufacturing a stepped drawn pipe having predetermined inner diameters and outer diameters in a plurality of locations. In the method, a die and a tap are fixed to be movable in a drawing direction and a steel pipe is drawn while being pressure-clamped by bearing surfaces facing each other.

In addition, FIG. 7 of Patent Document 2 discloses a method of manufacturing a variable wall thickness steel pipe using a die and a plug each having two steps of diameters. The method includes a step of forming a base steel pipe restricted in size by a bearing diameter  $d_2$  (small diameter) of the die and a bearing diameter  $d_3$  (small diameter) of the plug, a step of forming a base steel pipe restricted in size by the bearing diameter  $d_2$  (small diameter) of the die and a bearing diameter  $d_4$  (large diameter) of the plug, and a step of forming a base steel pipe restricted in size by a bearing diameter  $d_1$  (large diameter) of the die and the bearing diameter  $d_4$  (large diameter) of the plug.

PRIOR ART DOCUMENT

Patent Document

[Patent Document 1] Japanese Unexamined Patent Application, First Publication No. S59-73115

[Patent Document 2] Japanese Unexamined Patent Application, First Publication No. 2012-16712

DISCLOSURE OF THE INVENTION

Problems to be Solved by the Invention

Incidentally, some vehicle body members or vehicle body components constituting a vehicle body of an automobile are obtained by performing bending with respect to a member having a hollow closed cross-sectional shape and partially forming a bent part. In variable wall thickness steel pipes obtained by manufacturing methods in Patent Document 1 or Patent Document 2, working is performed with respect to an entire raw pipe in a longitudinal direction. Accordingly, the entirety is in a work-hardened state. In order to perform

## 2

bending or the like with respect to such a variable wall thickness steel pipe which has been entirely work-hardened, there is a need to soften the work-hardening of variable wall thickness steel pipe by performing heat treatment in advance. If such heat treatment becomes unnecessary, considerable labor-saving can be expected when a variable wall thickness steel pipe is worked into a vehicle body member. In addition, since heat treatment is omitted, degeneration in the steel structure of the variable wall thickness steel pipe can also be prevented.

The present invention has been made in consideration of the foregoing circumstances and an object thereof is to provide a variable wall thickness steel pipe and a method of manufacturing a variable wall thickness steel pipe, in which a working amount at the time of manufacturing is small and heat treatment such as annealing becomes unnecessary when post-working such as bending is performed.

Means For Solving the Problem

In order to achieve the object, the present invention employs each of the following aspects.

(1) According to an aspect of the present invention, there is provided a method of manufacturing a variable wall thickness steel pipe with a hollow tubular raw pipe. The method includes locking the raw pipe in a die by thrusting a plug into the raw pipe from an one end side so as to expand an outer shape on the one end side, in a state where the raw pipe is disposed inside the die and movement of the raw pipe in a longitudinal direction is restricted; and performing ironing in which an inner shape of the raw pipe is expanded while the outer shape is maintained so that a thin portion is formed by further thrusting the plug toward the other end side of the raw pipe while the locked state of the raw pipe is maintained, whereas the restriction on the raw pipe is relaxed.

(2) In the method of manufacturing a variable wall thickness steel pipe according to (1), in the performing ironing, an unprocessed portion may remain on the other end side of the raw pipe by stopping thrusting the plug in the middle.

(3) In the method of manufacturing a variable wall thickness steel pipe according to (1) or (2), a thickness reduction rate of the thin portion in the performing ironing may be within a range from 10% to 90%.

(4) In the method of manufacturing a variable wall thickness steel pipe according to any one of (1) to (3), the plug used in the locking and the performing ironing may include a tip end portion having an outer shape size smaller than an inner shape size of the raw pipe, a base end portion having an outer shape size larger than the inner shape size of the raw pipe and smaller than an outer shape size of the raw pipe, and a tapered portion being provided between the tip end portion and the base end portion to be tapered from the base end portion toward the tip end portion.

(5) In the method of manufacturing a variable wall thickness steel pipe according to any one of (1) to (3), the plug used in the locking and the performing ironing may include a base end portion having an outer shape size larger than an inner shape size of the raw pipe and smaller than an outer shape size of the raw pipe, and a tip end portion leading to a tip end side of the base end portion and being tapered as being separated from the base end portion.

(6) In the method of manufacturing a variable wall thickness steel pipe according to (4) or (5), the base end portion may have a large-sized base end portion being disposed on the tip end portion side, and a small-sized base

end portion having an outer shape size smaller than an outer shape size of the large-sized base end portion.

(7) According to another aspect of the present invention, there is provided a method of manufacturing a variable wall thickness steel pipe with a hollow tubular raw pipe. The method includes locking the raw pipe in a die by thrusting a first plug into the raw pipe from one end side, so as to expand an outer shape size on the one end side, in a state where the raw pipe is disposed inside the die and movement of the raw pipe in a longitudinal direction is restricted; pulling the first plug from the raw pipe; and performing ironing in which an inner shape of the raw pipe is expanded while an outer shape of the raw pipe is maintained so that a thin portion is formed by thrusting a second plug, which has an outer shape different from the outer shape of the first plug, from the one end side of the raw pipe toward the other end side while the locked state of the raw pipe is maintained, whereas the restriction on the raw pipe is relaxed.

(8) In the method of manufacturing a variable wall thickness steel pipe according to (7), the second plug used in the performing ironing may include a small-sized tip end portion smaller than an inner shape size of the raw pipe, an intermediate-sized portion having an outer shape size larger than the inner shape size of the raw pipe, a large-sized portion having an outer shape size larger than the outer shape size of the intermediate-sized portion and smaller than an outer shape size of the raw pipe, a first tapered portion being provided between the small-sized tip end portion and the intermediate-sized portion, and a second tapered portion being provided between the intermediate-sized portion and the large-sized portion.

(9) In the method of manufacturing a variable wall thickness steel pipe according to (7), the second plug used in the performing ironing may include a base end portion having an outer shape size larger than the inner shape size of the raw pipe and smaller than an outer shape size of the raw pipe, and a third tapered portion being tapered from the base end portion toward a tip end portion.

(10) In the method of manufacturing a variable wall thickness steel pipe according to any one of (1) to (9), the die may include a hollow small-sized portion having an inner shape size corresponding to the outer shape size of the raw pipe, a hollow large-sized portion having an inner shape size larger than the outer shape size of the raw pipe, and a hollow tapered portion being provided between the hollow small-sized portion and the hollow large-sized portion and being tapered from the hollow large-sized portion toward the hollow small-sized portion.

(11) In the method of manufacturing a variable wall thickness steel pipe according to (10), the die may further include a hollow intermediate-diameter portion being provided in a part of the hollow small-sized portion in the longitudinal direction and having an inner shape size larger than the outer shape size of the raw pipe.

(12) The method of manufacturing a variable wall thickness steel pipe according to any one of (1) to (11) may further include drawing the raw pipe after performing ironing.

(13) According to another aspect of the present invention, there is provided a method of manufacturing a variable wall thickness steel pipe with a hollow tubular raw pipe. The method includes locking the raw pipe in a die by simultaneously or alternately thrusting plugs into the raw pipe respectively from one end side and the other end side of the raw pipe, so as to expand an outer shape on the one end side and an outer shape on the other end side; pulling the plug on the other end side while the plug is inserted on the one end

side; performing first ironing in which an inner shape of the raw pipe is expanded while the outer shape is maintained so that a first thin portion is formed by further thrusting the plug, which is inserted on the one end side, toward the other end side of the raw pipe while the one end side is locked in the die; inserting and pulling the plugs such that the plug is inserted on the other end side, whereas the plug on the one end side is pulled out; and performing second ironing in which the inner shape of the raw pipe is expanded while the outer shape is maintained so that a second thin portion is formed by further thrusting the plug on the other end side toward the one end side of the raw pipe while the other end side is locked in the die. In the locking, the raw pipe freely moves in a longitudinal direction of the raw pipe in a case where the plugs are simultaneously thrust, and movement of the raw pipe in a thrusting direction of the plugs is restricted in a case where the plugs are alternately thrust.

(14) The method of manufacturing a variable wall thickness steel pipe according to (13) may further include drawing the raw pipe after performing second ironing.

(15) In the method of manufacturing a variable wall thickness steel pipe according to any one of (1) to (14), the raw pipe may be a seamless steel pipe.

(16) According to an aspect of the present invention, there is provided a variable wall thickness steel pipe which employs the following configuration including an expanded portion that is provided on one side in a longitudinal direction and has a largest outer shape size in a case of being seen in a cross section perpendicular to the longitudinal direction, and a thin portion that is provided on the other side of the expanded portion in a case of being seen in the longitudinal direction and has a thickness smaller than a thickness of the expanded portion. In a case where an average value of hardness of the expanded portion is H1 and an average value of hardness of the thin portion is H2, H2>H1 may be satisfied.

As a way of obtaining each of the average values of hardness according to the specification of this application, the average value is obtained by measuring hardness of five spots on a part of a manufactured variable wall thickness steel pipe at a central position in a thickness direction at intervals of 1 mm in the longitudinal direction of the same variable wall thickness steel pipe, and calculating the average value of hardness of the five spots. In a case where it is difficult to obtain five measurement spots due to the small size, hardness of five spots may be measured at intervals of 1 mm in the circumferential direction of the variable wall thickness steel pipe, and the average value of the five spots may be calculated and used.

(17) The variable wall thickness steel pipe according to (16) may employ the following configuration further including a thick portion that is disposed on the other side of the thin portion in a case of being seen in the longitudinal direction and has a thickness greater than the thickness of the thin portion. In a case where an average value of hardness of the thick portion is H3, H2>H1≥H3 may be satisfied.

(18) The variable wall thickness steel pipe according to (17) may employ the following configuration. The thin portion includes a straight pipe portion having a smallest thickness in the thin portion, a first tapered portion being provided between the straight pipe portion and the expanded portion and having an outer shape expanded toward the expanded portion, and a second tapered portion being provided between the straight pipe portion and the thick portion and having a thickness increasing toward the thick portion. In a case where an average value of hardness of the first tapered portion is H4, an average value of hardness of the

straight pipe portion is H5, and an average value of hardness of the second tapered portion is H6, both expressions  $H5 > H6 \geq H3$  and  $H5 > H4 > H1$  may be satisfied.

(19) In the variable wall thickness steel pipe according to any one of (16) to (18), the thickness of the thin portion may be partially increased in a case of being seen in the longitudinal direction.

(20) In the variable wall thickness steel pipe according to (16), combinations of the expanded portions and the thin portions may be symmetrically provided at both ends in the longitudinal direction.

(21) The variable wall thickness steel pipe according to (20) may employ the following configuration further including a thick portion that is disposed between a pair of the thin portions and has a thickness greater than the thickness of the thin portion. In a case where an average value of hardness of the thick portion is H7,  $H2 > H1 \geq H7$  may be satisfied.

(22) According to another aspect of the present invention, there is provided a variable wall thickness steel pipe which employs the following configuration including a thick portion that is provided on one side in a longitudinal direction and has a greatest thickness in a case of being seen in a cross section perpendicular to the longitudinal direction, and a thin portion that is provided on the other side of the thick portion and has a thickness smaller than the thickness of the thick portion. An outer shape size in the longitudinal direction is constant. In a case where an average value of hardness of the thick portion is H8 and an average value of hardness of the thin portion is H9,  $H9 > H8$  is satisfied.

(23) In the variable wall thickness steel pipe according to any one of (16) to (22), in a case where the thin portion is seen in a circumferential direction of the thin portion in a cross section perpendicular to the longitudinal direction, the thin portion may have a rotationally symmetric shape in which regions having a relatively small thickness and relatively high hardness and regions having a relatively great thickness and relatively low hardness alternate with each other in the circumferential direction.

(24) In the variable wall thickness steel pipe according to any one of (16) to (23), a seamless steel pipe may be used as a material.

As the various types of hardness above, for example, Vickers hardness may be used.

#### Effects of the Invention

According to the present invention, for example, in the method of manufacturing a variable wall thickness steel pipe according to (1), it is possible to perform ironing in which the inner shape is expanded while the outer shape of the raw pipe is maintained by thrusting the plug into the raw pipe from one end side while the outer shape of the raw pipe on one end side is expanded and the raw pipe is locked in the die. Thus, the working amount to be applied to one end side of the raw pipe can be reduced to a working amount as small as the outer shape size thereof is expanded. Therefore, since work-hardening is small on one end side of the raw pipe, heat treatment such as annealing can be made unnecessary when post-working such as bending is performed.

In addition, since ironing is performed by thrusting the plug into the raw pipe while one end side of the raw pipe is locked in the die, there is no need to fix the raw pipe itself to the die, and ironing can be carried out by only relatively moving the plug with respect to the die.

Therefore, in the method of manufacturing a variable wall thickness steel pipe according to the aspect of the present invention, it is possible to easily manufacture a variable wall

thickness steel pipe in which a part having a great thickness on one end side and a thin portion subjected to ironing are formed.

Particularly, in the method of manufacturing a variable wall thickness steel pipe according to (2), since an unprocessed portion having a zero working amount can remain on the other end side of the raw pipe, heat treatment such as annealing can be made unnecessary when post-working such as bending is performed with respect to the unprocessed portion.

In addition, in the method of manufacturing a variable wall thickness steel pipe according to (7), for example, two regions, of which the inner shape sizes are different from each other, can be provided inside the thin portion, and it is possible to manufacture a variable wall thickness steel pipe in which the thickness and strength vary in stages in the longitudinal direction.

#### BRIEF DESCRIPTION OF THE DRAWINGS

FIG. 1 is a process drawing showing a method of manufacturing a variable wall thickness steel pipe according to a first embodiment of the present invention and is a cross-sectional view seen in a cross section including an axis of a raw pipe.

FIG. 2 is a view showing an example of a variable wall thickness steel pipe manufactured by the method of manufacturing a variable wall thickness steel pipe of the same embodiment and is a cross-sectional view seen in a cross section including the axis.

FIG. 3 is a view showing another example of a variable wall thickness steel pipe manufactured by the method of manufacturing a variable wall thickness steel pipe of the same embodiment and is a cross-sectional view seen in a cross section including the axis.

FIG. 4 is a process drawing showing a method of manufacturing a variable wall thickness steel pipe according to a second embodiment of the present invention and is a cross-sectional view seen in a cross section including an axis of a raw pipe.

FIG. 5 is a process drawing showing a subsequent process of the method of manufacturing a variable wall thickness steel pipe according to the same embodiment and is a cross-sectional view seen in a cross section including the axis of the raw pipe.

FIG. 6 is a view showing a variable wall thickness steel pipe manufactured by the method of manufacturing a variable wall thickness steel pipe according to the same embodiment and is a cross-sectional view seen in a cross section including the axis.

FIG. 7 is a process drawing showing a method of manufacturing a variable wall thickness steel pipe according to a third embodiment of the present invention and is a cross-sectional view seen in a cross section including an axis of a raw pipe.

FIG. 8 is a process drawing showing a method of manufacturing a variable wall thickness steel pipe according to a fourth embodiment of the present invention and is a cross-sectional view seen in a cross section including an axis of a raw pipe.

FIG. 9 is a view showing a variable wall thickness steel pipe manufactured by the method of manufacturing a variable wall thickness steel pipe according to the same embodiment and is a cross-sectional view seen in a cross section including the axis of the raw pipe.

FIG. 10 is a process drawing showing a method of manufacturing a variable wall thickness steel pipe according

to a fifth embodiment of the present invention and is a cross-sectional view seen in a cross section including an axis of a raw pipe.

FIG. 11 is a view showing an example of a variable wall thickness steel pipe manufactured by the method of manufacturing a variable wall thickness steel pipe according to the same embodiment and is a cross-sectional view seen in a cross section including the axis of the raw pipe.

FIG. 12 is a view showing another example of a variable wall thickness steel pipe manufactured by the method of manufacturing a variable wall thickness steel pipe according to the same embodiment and is a cross-sectional view seen in a cross section including the axis of the raw pipe.

FIG. 13 is a process drawing showing a method of manufacturing a variable wall thickness steel pipe according to a sixth embodiment of the present invention and is a cross-sectional view seen in a cross section including an axis of a raw pipe.

FIG. 14 is a view showing an example of a variable wall thickness steel pipe manufactured by the method of manufacturing a variable wall thickness steel pipe according to the same embodiment and is a cross-sectional view seen in a cross section including the axis of the raw pipe.

FIG. 15 is a view showing another example of a variable wall thickness steel pipe manufactured by the method of manufacturing a variable wall thickness steel pipe according to the same embodiment and is a cross-sectional view seen in a cross section including the axis of the raw pipe.

FIG. 16 is a process drawing showing a method of manufacturing a variable wall thickness steel pipe according to a seventh embodiment of the present invention and is a cross-sectional view seen in a cross section including an axis of a raw pipe.

FIG. 17 is a process drawing showing a method of manufacturing a variable wall thickness steel pipe according to an eighth embodiment of the present invention and is a cross-sectional view seen in a cross section including an axis of a raw pipe.

FIG. 18 is a view showing a variable wall thickness steel pipe manufactured by the method of manufacturing a variable wall thickness steel pipe of the same embodiment and is a cross-sectional view seen in a cross section including the axis of the raw pipe.

FIG. 19 is a schematic perspective view of a plug used in a method of manufacturing a variable wall thickness steel pipe according to a ninth embodiment of the present invention.

FIG. 20 is a view showing examples of variable wall thickness steel pipes manufactured by the same embodiment and is a cross-sectional view in which a middle portion is seen in a cross section orthogonal to its longitudinal direction.

## EMBODIMENTS OF THE INVENTION

A variable wall thickness steel pipe and a method of manufacturing a variable wall thickness steel pipe according to each of embodiments of the present invention will be described below with reference to the drawings. In each of the embodiments, a raw pipe 1 having tensile strength of 290 MPa or higher is preferably used as a material.

### First Embodiment

A method of manufacturing a variable wall thickness steel pipe according to the first embodiment includes a step of forming a diameter-increasing portion by performing pipe

expanding with respect to a part on one end side of a raw pipe using a die and a plug, and a step of ironing a middle portion on the other end side of the diameter-increasing portion such that the inner diameter of the raw pipe is increased while the outer diameter is maintained. Examples of a raw pipe as a working target in the present embodiment can include a hollow tubular metal pipe. Particularly, a round steel pipe is preferably used. As the round steel pipe, any of a seamless steel pipe, a UO pipe, a spiral pipe, and an electric resistance welded steel pipe can be applied.

Next, the die and the plug used in the manufacturing method of the present embodiment will be described with reference to FIGS. 1(a) to 1(c). A die 11 according to the present embodiment includes a die main body 11d. Inside the die main body 11d, a hollow small-diameter portion 11a having an inner diameter corresponding to an outer diameter  $d_1$  of the raw pipe 1, a hollow large-diameter portion 11b having an inner diameter larger than the outer diameter  $d_1$  of the raw pipe 1, and a tapered portion 11c being provided between the hollow small-diameter portion 11a and the hollow large-diameter portion 11b are formed. The hollow small-diameter portion 11a, the hollow large-diameter portion 11b, and the tapered portion 11c communicate with each other inside the die main body 11d. The “inner diameter corresponding to the outer diameter  $d_1$  of the raw pipe 1” indicates an inner diameter size in which a gap size to the extent that the raw pipe 1 can be taken out and put in with respect to the inside and the outside of the hollow small-diameter portion 11a is added to the outer diameter  $d_1$  of the raw pipe 1.

A tapered portion 21c of a plug 21 in FIGS. 1(a) to 1(c) has an outer circumferential surface forming a taper angle  $\theta$  based on a line parallel to an axis CL in a case of being seen in a cross section including the axis CL of the plug 21. It is preferable that the taper angle  $\theta$  is within a range from 1 to 40 degrees. If the taper angle  $\theta$  is smaller than 1 degree, snapping of the plug 21 in its entirety with respect to the raw pipe 1 becomes significant, so that a required working force becomes excessive. Meanwhile, if the taper angle  $\theta$  exceeds 40 degrees, a local surface pressure generated in the tapered portion 21c of the plug 21 at the time of thinning becomes excessive, so that there is a possibility that deterioration of a life span of the plug 21 will be caused.

The plug 21 according to the present embodiment is configured to include a small-diameter tip end portion 21a corresponding to an inner diameter  $d_2$  of the raw pipe 1, a large-diameter base end portion 21b having a diameter larger than the inner diameter  $d_2$  of the raw pipe 1 and a diameter smaller than the inner diameter of the hollow small-diameter portion 11a of the die 11, and the tapered portion 21c being provided between the small-diameter tip end portion 21a and the large-diameter base end portion 21b. The outer diameter of the large-diameter base end portion 21b is set to have a size smaller than the inner diameter  $d_1$  of the hollow small-diameter portion 11a of the die 11.

In order to manufacture a variable wall thickness steel pipe according to the present embodiment, first, as shown in FIG. 1(a), the raw pipe 1 is coaxially inserted into the die 11. At this time, positional alignment is performed such that one end portion 1a of the raw pipe 1 is positioned inside the hollow large-diameter portion 11b of the die 11. Then, each of the die 11 and the raw pipe 1 are in a fixed state. That is, the die 11 is in a state fixed to a base (not shown). In addition, the raw pipe 1 is stemmed such that an end portion of the raw pipe 1 on the sheet left side does not further move forward to the sheet left side. Accordingly, the relative

position of the raw pipe 1 with respect to the die 11 in a longitudinal direction is fixed.

After the raw pipe 1 is fixed inside the die 11, the small-diameter tip end portion 21a of the plug 21 is inserted from the one end portion 1a side of the raw pipe 1 toward a hollow portion 1b of the raw pipe 1.

Next, as shown in FIG. 1(b), as a diameter-increasing step, while the die 11 and the raw pipe 1 are in a fixed state, the tapered portion 21c and the large-diameter base end portion 21b of the plug 21 are thrust into the one end portion 1a of the raw pipe 1. The plug 21 is thrust until the tapered portion 21c reaches the position of the tapered portion 11c of the die 11. In this manner, until the tapered portion 21c reaches the position of the tapered portion 11c of the die 11, the relative position of the raw pipe 1 with respect to the die 11 is continuously fixed. Therefore, the raw pipe 1 is not pushed out from the die 11 by the tapered portion 21c.

For example, it is possible to manage whether or not the tapered portion 21c has reached the position of the tapered portion 11c by measuring the amount of a thrusting stroke of the plug 21 or reaction increasing in response to a thrust of the plug 21.

At the point of time of FIG. 1(a), when the raw pipe 1 is disposed inside the die 11, the one end portion 1a of the raw pipe 1 is positioned inside the hollow large-diameter portion 11b of the die 11. Therefore, there is a gap s between the hollow large-diameter portion 11b of the die 11 and the one end portion 1a of the raw pipe 1. If the plug 21 is thrust from this state as illustrated in FIG. 1(b), the one end portion 1a of the raw pipe 1 is increased in diameter by the tapered portion 21c and the large-diameter base end portion 21b of the plug 21. Accordingly, the gap s is gradually reduced, and the outer circumferential surface of the one end portion 1a eventually abuts on the inner circumferential surface of the tapered portion 11c of the die 11 and the inner circumferential surface of the hollow large-diameter portion 11b. In this manner, a straight pipe-shaped diameter-increasing portion 1c and a lock portion 1e1 leading to the diameter-increasing portion 1c are formed in the one end portion 1a of the raw pipe 1. The lock portion 1e1 forms a part of a middle portion 1e and has a tapered truncated conical shape having a tapered surface in tight contact with the tapered portion 11c of the die 11 as the outer circumferential surface.

When the diameter-increasing portion 1c is formed, a slight pulling strain is applied to the one end portion 1a of the raw pipe 1 in the circumferential direction.

Next, as shown in FIG. 1(c), as an ironing step, in a state where the fixed state of the raw pipe 1 is released, whereas the fixed state of the die 11 is maintained, the plug 21 is further thrust toward the other end portion 1d side of the raw pipe 1. That is, as shown in FIG. 1(b), after the diameter-increasing portion 1c is formed, the stemmed state of the raw pipe 1 toward the end portion on the sheet left side is released. Thereafter, thrusting of the plug 21 further proceeds. As the plug 21 is further thrust, the raw pipe 1 is pushed from the one end portion 1a toward the other end portion 1d side. However, since the lock portion 1e1 formed in the raw pipe 1 in the previous step remains locked in the tapered portion 11c of the die 11, the raw pipe 1 does not move.

As the plug 21 is further thrust, the large-diameter base end portion 21b of the plug 21 is thrust toward the other end portion 1d side of the raw pipe 1. In the middle portion 1e of the raw pipe 1 in which the large-diameter base end portion 21b of the plug 21 is thrust, the original inner diameter  $d_2$  of the raw pipe 1 is increased to a size corresponding to the diameter of the large-diameter base end

portion 21b of the plug 21. On the other hand, since the middle portion 1e of the raw pipe 1 is positioned inside the hollow small-diameter portion 11a of the die 11 and its outer diameter size is restricted due to the surroundings, the outer diameter  $d_1$  of the middle portion 1e is not increased. Therefore, the middle portion 1e of the raw pipe 1 is subjected to ironing while the original outer diameter  $d_1$  of the raw pipe 1 is maintained.

The reason for releasing the stemmed state of the raw pipe 1 immediately before ironing starts is that a flow of the thickness of the raw pipe 1 entailed in ironing is not to be hindered. That is, when the middle portion 1e of the raw pipe 1 is reduced in thickness through ironing, in order to ensure as much room for the quantity as thickness reduction, the stemmed state of the raw pipe 1 is released. Accordingly, a part of the raw pipe 1 on the sheet left side is prevented from being buckled. In the present embodiment, since the quantity of thickness reduction of the raw pipe 1 due to ironing flows toward the sheet left side, the entire length of the raw pipe 1 becomes slightly longer than that before working.

In order to achieve an effect of improving strength of the middle portion 1e due to ironing, the thickness reduction rate of the raw pipe 1 due to ironing is required to be 10% or higher. Meanwhile, if the thickness reduction rate of the raw pipe 1 due to ironing exceeds 90%, there is concern that a fracture, burning, or the like is caused. Therefore, it is favorable that the thickness reduction rate of the raw pipe 1 due to ironing is within a range from 10% to 90%. Preferably, it is favorable that the thickness reduction rate is within a range from 20% to 80%. When the thickness of the raw pipe 1 before ironing is  $d_0$  and the thickness of the middle portion 1e after ironing is  $d$ , the thickness reduction rate (%) is expressed by  $(d_0-d)/d_0 \times 100\%$ .

Here, in a case where the thickness  $d$  of the middle portion 1e after ironing is not uniform when seen in the longitudinal direction of the raw pipe 1, and there is a distribution, the numerical value obtained in a location having the greatest amount of thickness reduction is employed as the thickness reduction rate. That is, in the middle portion 1e, the value obtained in a location in which the difference (equivalent strain amount) obtained by subtracting  $d$  from  $d_0$  is the greatest in a case of being seen in its longitudinal direction is employed as the thickness reduction rate described above. Furthermore, in a case where the amount of thickness reduction is not uniform in the circumferential direction of the raw pipe 1 and there is a distribution, the value obtained in a location in which the amount of thickness reduction is the greatest in the distribution in the circumferential direction is employed as the thickness reduction rate described above.

The thickness reduction rate can be adjusted by changing the diameter of the large-diameter base end portion 21b of the plug 21. The above-described appropriate range related to the thickness reduction rate in ironing is the same in other embodiments to be described below.

In the example shown in FIG. 1(c), the tapered portion 21c and the large-diameter base end portion 21b of the plug 21 are thrust to a position in front of the other end portion 1d of the raw pipe 1. If thrusting of the plug 21 stops at the position as illustrated in FIG. 1(c), a part on the other end portion 1d side of the middle portion 1e of the raw pipe 1 remains unprocessed. In this specification, a part that "remains unprocessed" denotes a part having substantially the same strength (tensile strength) or hardness of the raw pipe 1 before working (base metal) in a variable wall thickness steel pipe.

FIG. 2 shows a schematic cross-sectional view of a variable wall thickness steel pipe 31 manufactured via the steps shown in FIGS. 1(a) to 1(c). In the description below, in order to distinguish the manufactured variable wall thickness steel pipe from the raw pipe 1 before working and during working in the description, the new reference sign 31 is allocated thereto. Similarly, the description will proceed while having new reference signs applied to portions constituting the variable wall thickness steel pipe 31. In order to clarify the correspondence relationship with respect to the portions constituting the raw pipe 1, there are cases where parenthesized reference signs are appended to portions at the point of time of the raw pipe 1. The same also applies to each of the embodiments to be described below.

The variable wall thickness steel pipe 31 shown in FIG. 2 is configured to include a diameter-increasing portion 31c (1c) which is located on one end portion 31a (1a) side and is increased in diameter from the raw pipe 1, a middle portion 31e (1e) which is located between the one end portion 31a and the other end portion 31d (1d) and is subjected to ironing, and an unprocessed portion 31f which is located on the other end portion 31d side of the middle portion 31e and remains unprocessed as the raw pipe 1. The middle portion 31e also includes a part subjected to working by the tapered portions 11c and 21c of the die 11 and the plug 21 at each of boundaries with respect to the diameter-increasing portion 31c and the unprocessed portion 31f. That is, in a case of being seen from the one end portion 31a toward the other end portion 31d, the middle portion 31e includes a lock portion 31e1 (1e1) having a constant inner diameter and a tapered outer diameter, a straight pipe portion 31e2 having an inner diameter and an outer diameter both of which are constant, and a tapered portion 31e3 having a constant outer diameter and a tapered inner diameter. Then, in a case where the average value of hardness of the diameter-increasing portion 31c is H1, the average value of hardness of the unprocessed portion 31f is H3, the average value of hardness of the lock portion 31e1 is H4, the average value of hardness of the straight pipe portion 31e2 is H5, and the average value of hardness of the tapered portion 31e3 is H6, both expressions  $H5>H6\geq H3$  and  $H5>H4>H1$  are satisfied.

In FIG. 2, for the description, the diameter-increasing portion 31c is shown to have a short ring shape. However, as necessary, the diameter-increasing portion 31c may have a long straight pipe shape. The same applies to each of a diameter-increasing portion 41c, a diameter-increasing portion 61c, a diameter-increasing portion 91c, diameter-increasing portions 111c and 111f, a diameter-increasing portion 121c, a diameter-increasing portion 141c, and a diameter-increasing portion 151c in other embodiments to be described below.

In the diameter-increasing portion 31c and the middle portion 31e, a hollow portion 31b of the variable wall thickness steel pipe 31 is further increased in diameter than the original inner diameter  $d_2$  of the raw pipe 1. In the unprocessed portion 31f, the original inner diameter  $d_2$  of the raw pipe 1 remains unchanged. In addition, the outer diameter of the variable wall thickness steel pipe 31 is gradually increased from the outer diameter  $d_1$  of the raw pipe 1 in the lock portion 31e1. Then, in the diameter-increasing portion 31c, the outer diameter thereof is constant while being further increased than the outer diameter  $d_1$  of the raw pipe 1. Meanwhile, a part excluding the lock portion 31e1 in the middle portion 31e, and the unprocessed portion 31f remain having an outer diameter equal to the outer diameter  $d_1$  of the raw pipe 1. Accordingly, the variable wall thickness steel

pipe 31 has a comparatively great thickness in the diameter-increasing portion 31c and the unprocessed portion 31f, and has a comparatively small thickness in the middle portion 31e.

In the variable wall thickness steel pipe 31 shown in FIG. 2, since a small working amount is applied to the diameter-increasing portion 31c and the unprocessed portion 31f, no work hardening has occurred in these parts, or even if work hardening has occurred, it is very insignificant. Therefore, the diameter-increasing portion 31c and the unprocessed portion 31f have comparatively low strength. Accordingly, even in a case where post-working such as bending is performed with respect to these parts, annealing treatment or the like for softening work hardening becomes unnecessary. In addition, since a large working amount is applied to the middle portion 31e of the variable wall thickness steel pipe 31, the middle portion 31e has comparatively high strength due to work hardening. That is, as seen in a hardness distribution (Vickers hardness distribution, determination can also be made through a tensile strength distribution instead of Vickers hardness distribution) in the longitudinal direction of the variable wall thickness steel pipe 31, the unprocessed portion 31f has the lowest hardness, and the diameter-increasing portion 31c has hardness slightly higher than hardness of the unprocessed portion 31f. Then, the middle portion 31e has hardness higher than hardness of the diameter-increasing portion 31c. Therefore, since the middle portion 31e has the highest hardness, it is preferable to be used for a portion requiring high mechanical strength. In addition, the unprocessed portion 31f and the diameter-increasing portion 31c having relatively low hardness are preferable to be used as portions requiring post-working such as bending.

In addition, the inner surface of the middle portion 31e has small surface roughness by being subjected to ironing. If the surface roughness is reduced, fatigue properties increase. Accordingly, in addition to improvement of strength due to work hardening, the middle portion 31e can also achieve improvement of fatigue properties due to the reduced surface roughness on the inner surface, thereby realizing weight reduction and high strength. Such a synergistic effect cannot be achieved in thinning through simple cutting.

In addition, FIG. 3 shows another example of a variable wall thickness steel pipe manufactured via the steps shown in FIGS. 1(a) to 1(c). A variable wall thickness steel pipe 41 shown in FIG. 3 is a variable wall thickness steel pipe manufactured by thrusting the plug 21 until the large-diameter base end portion 21b of the plug 21 reaches the other end portion 1d of the raw pipe 1, in the step shown in FIG. 1(c).

The variable wall thickness steel pipe 41 shown in FIG. 3 is configured to include the diameter-increasing portion 41c (1c) which is located on one end portion 41a side and is increased in diameter from the raw pipe 1, a middle portion 41e (1e) which is located between the one end portion 41a (1a) and the other end portion 41d (1d) and is subjected to ironing, and the other end part 41f which is located on the other end portion 41d side of the middle portion 41e and is subjected to ironing, similar to the middle portion 41e. The middle portion 41e also includes a part subjected to working by the tapered portion 11c of the die 11 and the tapered portion 21c of the plug 21 at a boundary with respect to the diameter-increasing portion 41c. That is, the middle portion 41e includes a lock portion 41e1 (1e1). Since the lock portion 41e1 has the same shape as the lock portion 31e1, a duplicate description thereof will be omitted herein.

In a hollow portion  $41b$  of the variable wall thickness steel pipe  $41$ , the entire inner diameter in its longitudinal direction is further increased than the inner diameter  $d_2$  of the raw pipe  $1$ . In addition, the outer diameter of the variable wall thickness steel pipe  $41$  is gradually increased from the outer diameter  $d_1$  of the raw pipe  $1$  in the lock portion  $41e1$ . Then, in the diameter-increasing portion  $41c$ , the outer diameter thereof is constant while being further increased than the outer diameter  $d_1$  of the raw pipe  $1$ . Meanwhile, a part excluding the lock portion  $41e1$  in the middle portion  $41e$ , and the other end part  $41f$  remain having an outer diameter equal to the outer diameter  $d_1$  of the raw pipe  $1$ . Accordingly, the variable wall thickness steel pipe  $41$  has a comparatively great thickness in the lock portion  $41e1$  and the diameter-increasing portion  $41c$  and has a comparatively small thickness in a part excluding the lock portion  $41e1$  in the middle portion  $41e$ , and the other end part  $41f$ .

In the variable wall thickness steel pipe  $41$  shown in FIG. 3, since a small working amount is applied to the diameter-increasing portion  $41c$ , no work hardening has occurred in this part, or even if work hardening has occurred, it is very insignificant. Therefore, the diameter-increasing portion  $41c$  has comparatively low strength. Accordingly, even in a case where post-working such as bending is performed with respect to this part, annealing treatment or the like for softening work hardening becomes unnecessary.

In addition, since a large working amount is applied to the middle portion  $41e$  and the other end part  $41f$  of the variable wall thickness steel pipe  $41$ , the middle portion  $41e$  and the other end part  $41f$  have comparatively high strength due to work hardening.

As described above, in the embodiment shown in FIGS. 1(a) to 2, the lock portion  $1e1$  and the diameter-increasing portion  $1c$  are provided by performing pipe expanding with respect to the one end portion  $1a$  of the raw pipe  $1$ , and ironing is performed with respect to the middle portion  $1e$  on the other end portion  $1d$  side of the diameter-increasing portion  $1c$  of the raw pipe  $1$  such that the inner diameter is increased while the outer diameter of the raw pipe  $1$  is maintained, by further thrusting the plug  $21$  into the raw pipe  $1$  while the lock portion  $1e1$  is locked inside the die  $11$ . Therefore, the working amount with respect to the diameter-increasing portion  $1c$  can be reduced, so that heat treatment such as annealing can be made unnecessary when post-working such as bending is performed with respect to the diameter-increasing portion  $1c$ .

In addition, since ironing is performed by thrusting the plug  $21$  into the raw pipe  $1$  while the diameter-increasing portion  $1c$  is locked in the die  $11$ , ironing can be carried out by only relatively moving the die  $11$  and the plug  $21$  without requiring labor and tools for fixing the raw pipe  $1$  itself.

In addition, since a part of the raw pipe  $1$  on the other end portion  $1d$  side of the middle portion  $1e$  is caused to be the unprocessed portion  $31f$  which remains unprocessed, the working amount with respect to a part on the other end portion  $1d$  side becomes zero, so that heat treatment such as annealing can be made unnecessary when post-working such as bending is performed with respect to the unprocessed portion  $31f$ .

In addition, in the variable wall thickness steel pipe  $31$  manufactured by the method described above, since the diameter-increasing portion  $31c$  and the unprocessed portion  $31f$  have a small working amount, the thickness is large and strength is comparatively low. Meanwhile, in the middle portion  $31e$ , since the working amount thereof is large, the thickness is small and strength is comparatively high. Therefore, the diameter-increasing portion  $31c$  and the unpro-

cessed portion  $31f$  are in a state where deformability remains, compared to the middle portion  $31e$ , and these parts form the variable wall thickness steel pipe  $31$  having excellent post-workability such as bending. In addition, since the middle portion  $31e$  has small inner surface roughness by being subjected to ironing, this part forms the variable wall thickness steel pipe  $31$  having excellent fatigue properties.

#### Second Embodiment

10

A method of manufacturing a variable wall thickness steel pipe of a second embodiment is configured to include a step of forming a diameter-increasing portion by performing pipe expanding with respect to a part on one end side of a raw pipe using a die and a plug, and a step of ironing a middle portion on the other end side of the diameter-increasing portion such that the inner diameter of the raw pipe is increased while the outer diameter is maintained after the plug is replaced with another plug. A raw pipe as a working target of the present embodiment may be similar to that of the first embodiment.

In the present embodiment, a die and a plug similar to those of the first embodiment are used in the step of forming the diameter-increasing portion, which is performed first.

That is, similar to the case of the first embodiment, as shown in FIG. 4(a), the raw pipe  $1$  is inserted into the die  $11$ , and positional alignment is performed such that the one end portion  $1a$  of the raw pipe  $1$  is positioned inside the hollow large-diameter portion  $11b$  of the die  $11$ . Each of the die  $11$  and the raw pipe  $1$  are in a fixed state. Then, the small-diameter tip end portion  $21a$  of the plug  $21$  is inserted into the hollow portion  $1b$  of the raw pipe  $1$  from the one end portion  $1a$  side of the raw pipe  $1$ .

Next, as shown in FIG. 4(b), as the diameter-increasing step, while the die  $11$  and the raw pipe  $1$  are in a fixed state, the tapered portion  $21c$  and the large-diameter base end portion  $21b$  of the plug  $21$  are thrust into the one end portion  $1a$  of the raw pipe  $1$ . The plug  $21$  is thrust until the tapered portion  $21c$  reaches the position of the tapered portion  $11c$  of the die  $11$ . Accordingly, similar to the first embodiment, the lock portion  $1e1$  and the diameter-increasing portion  $1c$  are formed in the one end portion  $1a$  of the raw pipe  $1$ .

Next, as shown in FIG. 4(c), the thrust plug  $21$  is pulled out from the raw pipe  $1$  to be replaced with another plug. Meanwhile, the die  $11$  is continuously used to the end without being replaced.

Next, as shown in FIG. 5(a), a different plug  $51$  is prepared. The different plug  $51$  includes a small-diameter tip end portion  $51a$  corresponding to the inner diameter  $d_2$  of the raw pipe  $1$ , an intermediate-diameter portion  $51b$  having a diameter larger than the inner diameter  $d_2$  of the raw pipe  $1$  or the outer diameter of the small-diameter tip end portion  $51a$ , a large-diameter base end portion  $51c$  having a diameter larger than the diameter of the intermediate-diameter portion  $51b$ , a first tapered portion  $51d$  being provided between the small-diameter tip end portion  $51a$  and the intermediate-diameter portion  $51b$ , and a second tapered portion  $51e$  being provided between the intermediate-diameter portion  $51b$  and the large-diameter base end portion  $51c$ . In addition, the diameter of the large-diameter base end portion  $51c$  is set to have a size smaller than the inner diameter  $d_1$  of the hollow small-diameter portion  $11a$  of the die  $11$ . In addition, the diameter of the small-diameter tip end portion  $51a$  of the plug  $51$  has the same size as the diameter of the small-diameter tip end portion  $21a$  of the plug  $21$  used previously.

Then, as shown in FIG. 5(b), as the ironing step, in a state where the fixed state of the raw pipe 1 is released, whereas the fixed state of the die 11 is maintained, the plug 51 is thrust from the one end portion 1a of the raw pipe 1 toward the other end portion 1d. As the plug 51 is thrust, the raw pipe 1 is pushed from the one end portion 1a toward the other end portion 1d side. However, since the lock portion 1e1 formed in the raw pipe 1 in the previous step remains locked in the tapered portion 11c of the die 11, the raw pipe 1 does not move. In the present embodiment, the plug 51 is thrust until the tip end of the small-diameter tip end portion 51a protrudes from the other end portion 1d of the raw pipe 1.

As the plug 51 is thrust to the position shown in FIG. 5(b), the intermediate-diameter portion 51b and the large-diameter base end portion 51c of the plug 51 are thrust into the middle portion 1e of the raw pipe 1. In the middle portion 1e of the raw pipe 1, the original inner diameter  $d_2$  of the raw pipe 1 is increased to a size corresponding to the diameters of the intermediate-diameter portion 51b and the large-diameter base end portion 51c of the plug 51. On the other hand, since the middle portion 1e of the raw pipe 1 is positioned inside the hollow small-diameter portion 11a of the die 11, the outer diameter  $d_1$  of the middle portion 1e is not increased. Therefore, the middle portion 1e of the raw pipe 1 is subjected to ironing while the original outer diameter  $d_1$  of the raw pipe 1 is maintained, excluding a part of the lock portion 1e1.

In addition, as shown in FIG. 5(b), a part on the other end portion 1d side of the middle portion 1e of the raw pipe 1 is only a part into which the small-diameter tip end portion 51a is inserted, so that the part remains unprocessed.

FIG. 6 shows a schematic cross-sectional view of a variable wall thickness steel pipe 61 manufactured via the steps shown in FIGS. 4(a) to 5(b). The variable wall thickness steel pipe 61 shown in FIG. 6 is configured to include the diameter-increasing portion 61c (1c) which is located on one end portion 61a side and is increased in diameter from the raw pipe 1, a middle portion 61e (1e) which is located between the one end portion 61a (1a) and the other end portion 61d (1d) and is subjected to ironing, and an unprocessed portion 61f which is located on the other end portion 61d side of the middle portion 61e and remains unprocessed as the raw pipe 1. The middle portion 61e also includes a part subjected to working by the tapered portion 11c of the die 11 and the tapered portions 51d and 51e of the plug 51 at each of boundaries with respect to the diameter-increasing portion 61c and the unprocessed portion 61f. That is, the middle portion 61e includes a lock portion 61e1 (1e1). Since the lock portion 61e1 has the same shape as the lock portion 31e1, a duplicate description thereof will be omitted herein.

In the diameter-increasing portion 61c and the middle portion 61e, the inner diameter of a hollow portion 61b of the variable wall thickness steel pipe 61 is further increased than the inner diameter  $d_2$  of the raw pipe 1. Then, in the unprocessed portion 61f, the inner diameter of a hollow portion 61b of the variable wall thickness steel pipe 61 remains the inner diameter  $d_2$  of the raw pipe 1. In addition, in the middle portion 61e, the inner diameter of a part on the one end portion 61a side is increased by the large-diameter base end portion 51c of the plug 51, and the inner diameter of a part on the other end portion 61d side is increased by the intermediate-diameter portion 51b of the plug 51. Furthermore, inner diameter of a part on the one end portion 61a side and the inner diameter of a part on the other end portion 61d side are different from each other. In addition, in the

lock portion 61e1 and the diameter-increasing portion 61c, the outer diameter of the variable wall thickness steel pipe 61 is further increased than the outer diameter  $d_1$  of the raw pipe 1. Meanwhile, the outer diameters of a part excluding the lock portion 61e1 in the middle portion 61e, and the unprocessed portion 61f remain unchanged as the outer diameter  $d_1$  of the raw pipe 1. Accordingly, the variable wall thickness steel pipe 61 has a comparatively great thickness in the diameter-increasing portion 61c and the unprocessed portion 61f and has a comparatively small thickness in the middle portion 61e.

In the variable wall thickness steel pipe 61 shown in FIG. 6, since a small working amount is applied to the diameter-increasing portion 61c and the unprocessed portion 61f, no work hardening has occurred in these parts, or even if work hardening has occurred, it is very insignificant. Therefore, the diameter-increasing portion 61c or the unprocessed portion 61f has comparatively low strength. Accordingly, even in a case where post-working such as bending is performed with respect to these parts, annealing treatment or the like for softening work hardening becomes unnecessary.

In addition, since a comparatively large working amount is applied to the middle portion 61e of the variable wall thickness steel pipe 61, the middle portion 61e has comparatively high strength due to work hardening.

In the present embodiment as described above, ironing is performed with respect to the middle portion 1e of the raw pipe 1 using the plug 51. In this case, in the middle portion 1e, the diameter-increasing amount of a region on the diameter-increasing portion 1c side is larger than the diameter-increasing amount of a region on the other end portion 1d side, so that two regions of which the inner diameters and strengths are different from each other can be provided inside the middle portion 1e.

In addition, the variable wall thickness steel pipe 61 manufactured by the method described above has the middle portion 61e in which the diameter-increasing amount of a region on the diameter-increasing portion 61c side is larger than the diameter-increasing amount of a region on the other end portion 61d side, and the working amount of a region on the diameter-increasing portion 61c side is larger than the working amount of a region on the other end portion 61d side. Therefore, the variable wall thickness steel pipe 61 has regions of which the thicknesses and strength are different from each other in the middle portion 61e.

### Third Embodiment

A method of manufacturing a variable wall thickness steel pipe of a third embodiment will be described with reference to FIGS. 7(a) to 7(c). The method of manufacturing a variable wall thickness steel pipe of the present embodiment is configured to include a step similar to that of the first embodiment. In the present embodiment, the variable wall thickness steel pipe is manufactured by using a plug 71 which is different from the plug 21 used in the first embodiment. Since other configurations are similar to those of the first embodiment, a description will be omitted.

As shown in FIG. 7(a), the plug 71 used in the present embodiment is configured to include a tapered tip end portion 71c having a tip end portion 71a smaller than the inner diameter  $d_2$  of the raw pipe 1, and a base end portion 71b having a diameter larger than the inner diameter  $d_2$  of the raw pipe 1. In addition, the diameter of the base end portion 71b is set to have a size smaller than the inner diameter  $d_1$  of the hollow small-diameter portion 11a of the die 11.

In the present embodiment, similar to the first embodiment, as shown in FIG. 7(b), as the diameter-increasing step, while the die 11 and the raw pipe 1 are in a fixed state, the tapered tip end portion 71c and the base end portion 71b of the plug 71 are thrust into the one end portion 1a of the raw pipe 1. The plug 71 is thrust until the tapered tip end portion 71c reaches the position of the tapered portion 11c of the die 11. Accordingly, the lock portion 1e1 and the diameter-increasing portion 1c are formed in the one end portion 1a of the raw pipe 1.

Next, as shown in FIG. 7(c), as the ironing step, in a state where the fixed state of the raw pipe 1 is released, whereas the fixed state of the die 11 is maintained, the plug 71 is further thrust toward the other end portion 1d side of the raw pipe 1. As the plug 71 is further thrust, the raw pipe 1 is pushed from the one end portion 1a toward the other end portion 1d side. However, since the lock portion 1e1 formed in the raw pipe 1 in the previous step remains locked in the tapered portion 11c of the die 11, the raw pipe 1 does not move.

Since the plug 71 in the present embodiment is configured to include the tapered tip end portion 71c and the base end portion 71b and does not include the small-diameter tip end portion 21a shown in the first embodiment, its length in the longitudinal direction is comparatively short. Therefore, compared to the first embodiment, the required stroke amount of the plug 71 when inserting the plug 71 into the raw pipe 1 or when pulling out the plug 71 from the raw pipe 1 becomes short. As a result, the work hour for taking out and putting in the plug 71 can be shortened, and a hydraulic cylinder (not shown) having a simple structure for taking out and putting in the plug 71 can be employed. Therefore, it is possible to perform working even with comparatively small manufacturing equipment.

The variable wall thickness steel pipe which has been manufactured via the steps shown in FIGS. 7(a) to 7(c) has a shape similar to that of the variable wall thickness steel pipe 31 shown in FIG. 2. In addition, in the step shown in FIG. 7(c), the variable wall thickness steel pipe may be worked into a shape similar to the variable wall thickness steel pipe 41 as shown in FIG. 3 by thrusting the plug 71 until the base end portion 71b of the plug 71 reaches the other end portion 1d of the raw pipe 1.

In the present embodiment as described above, since the variable wall thickness steel pipe is manufactured by using the plug 71 having a comparatively short length in the longitudinal direction, compared to the first embodiment, it is possible to comparatively reduce the required stroke amount of the plug 71 at the time of manufacturing.

#### Fourth Embodiment

Next, a method of manufacturing a variable wall thickness steel pipe of a fourth embodiment will be described. The method of manufacturing a variable wall thickness steel pipe of the present embodiment is configured to include a step similar to that of the second embodiment. In the present embodiment, ironing is performed by using a plug 81 different from the plug 51 used in the ironing step of the second embodiment. Since other configurations are similar to those of the second embodiment, a description will be omitted.

First, in the present embodiment, similar to the second embodiment, the lock portion 1e1 and the diameter-increasing portion 1c are formed in the raw pipe 1. Next, as shown in FIG. 8(a), the plug 81 different from that in the previous step is prepared. The plug 81 is configured to include a

tapered tip end portion 81c having a tip end portion 81a smaller than the inner diameter  $d_2$  of the raw pipe 1, and a base end portion 81b having a diameter larger than the inner diameter  $d_2$  of the raw pipe 1 and a diameter smaller than the inner diameter  $d_1$  of the hollow small-diameter portion 11a of the die 11. The tapered tip end portion 81c of the plug 81 is longer than the length of the tapered tip end portion 71c of the plug 71 shown in FIG. 7(a).

Then, as shown in FIG. 8(b), as the ironing step, in a state where the fixed state of the raw pipe 1 is released, whereas the fixed state of the die 11 is maintained, the plug 81 is thrust from the one end portion 1a of the raw pipe 1 toward the other end portion 1d. As the plug 81 is thrust, the raw pipe 1 is pushed from the one end portion 1a toward the other end portion 1d side. However, since the lock portion 1e1 formed in the raw pipe 1 in the previous step remains locked in the tapered portion 11c of the die 11, the raw pipe 1 does not move. In the present embodiment, the plug 81 is thrust until the tip end portion 81a of the plug 81 protrudes from the other end portion 1d of the raw pipe 1.

As the plug 81 is thrust to the position shown in FIG. 8(b), the tapered tip end portion 81c of the plug 81 is thrust into the middle portion 1e of the raw pipe 1. In the middle portion 1e of the raw pipe 1, the original inner diameter  $d_2$  of the raw pipe 1 is increased to a size corresponding to the diameter of the tapered tip end portion 81c of the plug 81.

Since the plug 81 used in the present embodiment includes the tapered tip end portion 81c having a comparatively long taper length, the inner diameter of the middle portion 1e of the raw pipe 1 becomes the same as the outer diameter of the tapered tip end portion 81c of the plug 81 over the entire length. That is, the inner diameter of the middle portion 1e of the raw pipe 1 is gradually increased from the other end portion 1d side to the one end portion 1a side.

FIG. 9 shows a schematic cross-sectional view of the variable wall thickness steel pipe manufactured in accordance with the present embodiment. A variable wall thickness steel pipe 91 shown in FIG. 9 is configured to include a diameter-increasing portion 91c (1c) which is located on one end portion 91a (1a) side and is increased in diameter from the raw pipe 1, a middle portion 91e (1e) which is located between the one end portion 91a and the other end portion 91d (1d) and is subjected to ironing, and an unprocessed portion 91f which is located on the other end portion 91d side of the middle portion 91e and remains unprocessed as the raw pipe 1.

In the diameter-increasing portion 91c and the middle portion 91e, the inner diameter of a hollow portion 91b of the variable wall thickness steel pipe 91 is further increased than the inner diameter  $d_2$  of the raw pipe 1. In the unprocessed portion 91f, the inner diameter  $d_2$  of the raw pipe remains unchanged. In addition, in a lock portion 91e1 and the diameter-increasing portion 91c, the outer diameter of the variable wall thickness steel pipe 91 is further increased than the outer diameter  $d_1$  of the raw pipe 1. A part excluding the lock portion 91e1 in the middle portion 91e, and the unprocessed portion 91f remain unchanged as the outer diameter  $d_1$  of the raw pipe 1. In addition, the inner diameter in the middle portion 91e gradually increases from the other end portion 1d side to the one end portion 1a side. Accordingly, the diameter-increasing portion 91c and the unprocessed portion 91f have a comparatively great thickness. In addition, in a case where the thickness of the middle portion 91e is seen from the diameter-increasing portion 91c toward the unprocessed portion 91f, the thickness is gradually

reduced in the lock portion **91e1** and gradually increases in parts other than the lock portion **91e1**.

In the variable wall thickness steel pipe **91** shown in FIG. 9, since a small working amount is applied to the diameter-increasing portion **91c** and the unprocessed portion **91f**, no work hardening has occurred in these parts, or even if work hardening has occurred, it is very insignificant.

In addition, in the middle portion **91e** of the variable wall thickness steel pipe **91**, since the working amount is gradually reduced from the diameter-increasing portion **91c** to the unprocessed portion **91f**, hardness is comparatively high on the diameter-increasing portion **91c** side of the middle portion **91e**, and hardness is comparatively low on the unprocessed portion **91f** side.

As described above, in the present embodiment, ironing is performed with respect to the middle portion **1e** of the raw pipe **1** by using the plug **81** having the tapered tip end portion **81c** which is comparatively long. Therefore, it is possible to manufacture the variable wall thickness steel pipe in which the inner diameter is gradually reduced from the diameter-increasing portion **1c** side to the other end portion **1d** side in the middle portion **1e**.

#### Fifth Embodiment

A method of manufacturing a variable wall thickness steel pipe of a fifth embodiment is configured to include a step of forming diameter-increasing portions **1c** and **1f** by performing pipe expanding with respect to both end parts of the raw pipe **1** using one die and two plugs; a step of performing first ironing in which a plug **22** on the other end side is pulled while the plug **21** on one end side is inserted in the raw pipe **1**, and the inner diameter of a middle portion **1g** on the other end side of the diameter-increasing portion **1c** on one end side is increased while the outer diameter of the raw pipe **1** is maintained; and a step of performing second ironing in which the plug **21** on one end side is pulled from the raw pipe **1**, the plug **22** on the other end side is inserted into the raw pipe **1**, and the inner diameter of a middle portion **1h** on one end side of the diameter-increasing portion **1f** on the other end side is increased while the outer diameter of the raw pipe **1** is maintained. The raw pipe **1** as a working target of the present embodiment may be similar to that of the first embodiment.

In the present embodiment, a die **12** shown in FIG. 10(a) is used. The die **12** is configured to include a hollow small-diameter portion **12b** having an inner diameter corresponding to the outer diameter **d<sub>1</sub>** of the raw pipe **1**, and a hollow large-diameter portion **12a** and a hollow large-diameter portion **12d** being provided on both sides of the hollow small-diameter portion **12b** in the longitudinal direction and having an inner diameter larger than the outer diameter **d<sub>1</sub>** of the raw pipe **1**. In addition, a tapered portion **12c** is provided between the hollow small-diameter portion **12b** and the hollow large-diameter portion **12a**, and a tapered portion **12e** is provided between the hollow small-diameter portion **12b** and the hollow large-diameter portion **12d**. The hollow large-diameter portion **12a**, the tapered portion **12c**, the hollow small-diameter portion **12b**, the tapered portion **12e**, and the hollow large-diameter portion **12d** communicate with each other inside a die main body **12f**. In addition, the die **12** has a two-division structure which can be divided in an upward/downward direction in FIG. 10(a).

The one-dot chained lines vertically shown in FIGS. 10(a) to 10(d) are center lines indicating half the length of the die

**12** in the longitudinal direction, and the die **12** has a line symmetric shape having this one-dot chained line as a symmetric axis.

Since the plug **21** shown in FIG. 10(a) is similar to that used in the first embodiment, the same reference sign is applied and description is omitted. The plug **22** has a shape similar to the plug **21** and is configured to include a small-diameter tip end portion **22a** corresponding to the inner diameter **d<sub>2</sub>** of the raw pipe **1**, a large-diameter base end portion **22b** having a diameter larger than the inner diameter **d<sub>2</sub>** of the raw pipe **1**, and a tapered portion **22c** being provided between the small-diameter tip end portion **22a** and the large-diameter base end portion **22b**. In addition, the diameter of the large-diameter base end portion **22b** is set to have a size smaller than the inner diameter **d<sub>1</sub>** of the hollow small-diameter portion **12b** of the die **12**.

In order to manufacture the variable wall thickness steel pipe according to the present embodiment, first, as shown in FIG. 10(a), the raw pipe **1** is inserted into the die **12**. At this time, positional alignment is performed such that the one end portion **1a** and the other end portion **1d** of the raw pipe **1** are respectively positioned in the hollow large-diameter portions **12a** and **12d** of the die **12**. Then, the small-diameter tip end portion **21a** of the plug **21** and the small-diameter tip end portion **22a** of the plug **22** are inserted into the hollow portion **1b** of the raw pipe **1** from the one end portion **1a** side and the other end portion **1d** side of the raw pipe **1**, respectively. At this time, the raw pipe **1** and the die **12** are in a non-fixed state.

Next, as the diameter-increasing step, as shown in FIG. 10(b), the tapered portion **21c** and the large-diameter base end portion **21b** of the plug **21** are thrust into the one end portion **1a** of the raw pipe **1**, and the tapered portion **22c** and the large-diameter base end portion **22b** of the plug **22** are thrust into the other end portion **1d** of the raw pipe **1**, simultaneously. In addition, the plug **21** is thrust until the tapered portion **21c** reaches the position of the tapered portion **12c** of the die **12**, and the plug **22** is thrust until the tapered portion **22c** reaches the position of the tapered portion **12e** of the die **12**. Accordingly, a lock portion **1g1** and the diameter-increasing portion **1c** are formed on the one end portion **1a** side of the raw pipe **1**. In addition, a lock portion **1h1** and the diameter-increasing portion **1f** are formed on the other end portion **1d** side.

Next, while the plug **21** on the one end portion **1a** side remains unchanged, the plug **22** on the other end portion **1d** side is pulled out from the raw pipe **1**. Thereafter, as shown in FIG. 10(c), as the first ironing step, while the fixed state of the raw pipe **1** is released, whereas the other end portion **12g** side of the die **12** is fixed, the plug **21** is further thrust toward the other end portion **1d** side of the raw pipe **1**. As the plug **21** is further thrust, the raw pipe **1** is pushed from the one end portion **1a** toward the other end portion **1d** side. However, since the lock portion **1g1** formed in the raw pipe **1** in the previous step remains locked in the tapered portion **12c** of the die **12**, the raw pipe **1** does not move.

In the example shown in FIG. 10(c), the tapered portion **21c** and the large-diameter base end portion **21b** of the plug **21** are thrust to the position on the one end portion **12h** side of a middle position of the die **12**. If thrusting of the plug **21** stops at the position as shown in FIG. 10(c), a part between the diameter-increasing portion **1f** of the raw pipe **1** on the other end portion **1d** side and a first working part **1g** of the raw pipe **1** subjected to ironing remains unprocessed.

Next, the plug **21** pulled out from the raw pipe **1**, and the plug **22** is inserted into the raw pipe **1** on the other end portion **1d** side. Then, as shown in FIG. 10(d), as the second

ironing step, the plug 22 is further thrust toward the one end portion 1a side of the raw pipe 1. At this time, the raw pipe 1 is in a non-fixed state, whereas the one end portion 12h side of the die is fixed. As the plug 22 is further thrust, the raw pipe 1 is pushed from the other end portion 1d side toward the one end portion 1a side. However, since the lock portion 1h1 formed in the raw pipe 1 in advance in the diameter-increasing step is locked in the tapered portion 12e of the die 12, the raw pipe 1 does not move.

In the example shown in FIG. 10(d), the tapered portion 22c and the large-diameter base end portion 22b of the plug 22 are thrust to the position on the other end portion 12g side of the middle of the die 12. If thrusting of the plug 22 stops at the position as shown in FIG. 10(d), a middle portion 1i between the first working part 1g and a second working part 1h of the raw pipe 1 remains unprocessed.

FIG. 11 shows a schematic cross-sectional view of a variable wall thickness steel pipe 111 manufactured via the steps shown in FIGS. 10(a) to 10(d). The variable wall thickness steel pipe 111 is configured to include the diameter-increasing portion 111c (1c) which is located on one end portion 111a (1a) side and is increased in diameter from the raw pipe 1, a first working part 111g (1g) which is located between the one end portion 111a and the other end portion 111d (1d) and is subjected to first ironing, the diameter-increasing portion 111f (1f) which is located on the other end portion 111d side and is increased in diameter from the raw pipe 1, a second working part 111h (1h) which is located between the other end portion 111d and the one end portion 111a and is subjected to second ironing, and an unprocessed portion 111i (1i) which is located between the first working part 111g and the second working part 111h and remains unprocessed as the raw pipe 1.

The first working part 111g also includes parts subjected to working by the tapered portions 12c and 21c of the die 12 and the plug 21 at each of boundaries with respect to the diameter-increasing portion 111c and the unprocessed portion 111i. That is, the first working part 111g includes a lock portion 111g1 (1g1) leading to the diameter-increasing portion 111c, and a tapered portion 111g2 leading to the unprocessed portion 111i.

The second working part 111h also includes parts subjected to working by the tapered portions 12c and 22c of the die 12 and the plug 22 at each of boundaries with respect to the diameter-increasing portion 111f and the unprocessed portion 111i. That is, the second working part 111h includes a lock portion 111h1 (1h1) leading to the diameter-increasing portion 111f, and a tapered portion 111h2 leading to the unprocessed portion 111i.

A hollow portion 111b of the variable wall thickness steel pipe 111 is further increased in diameter than the original inner diameter  $d_2$  of the raw pipe 1 in the diameter-increasing portion 111c, the first working part 111g, the diameter-increasing portion 111f, and the second working part 111h. Meanwhile, in the unprocessed portion 111i, the original inner diameter  $d_2$  of the raw pipe 1 remains unchanged. In addition, the outer diameter of the variable wall thickness steel pipe 111 is further increased than the outer diameter  $d_1$  of the raw pipe 1 in the diameter-increasing portion 111c, a lock portion 111g1, the diameter-increasing portion 111f, and the lock portion 111h1. Meanwhile, a part excluding the lock portion 111g1 in the first working part 111g, a part excluding the lock portion 111h1 in the second working part 111h, and the unprocessed portion 111i remain unchanged as the outer diameter  $d_1$  of the raw pipe 1.

In addition, in regard to the thickness, the variable wall thickness steel pipe has a comparatively great thickness in

the diameter-increasing portion 111c, the diameter-increasing portion 111f, and the unprocessed portion 111i and has a comparatively small thickness in the first working part 111g and the second working part 111h.

In the variable wall thickness steel pipe 111 shown in FIG. 11, since a small working amount is applied to the diameter-increasing portion 111c, the diameter-increasing portion 111f, and the unprocessed portion 111i, no work hardening has occurred in these parts, or even if work hardening has occurred, it is very insignificant. Therefore, the diameter-increasing portion 111c, the diameter-increasing portion 111f, and the unprocessed portion 111i have comparatively low strength. Accordingly, even in a case where post-working such as bending is performed with respect to these parts, annealing treatment or the like for softening work hardening becomes unnecessary.

In addition, since a comparatively large working amount is applied to the first working part 111g and the second working part 111h, the first working part 111g and the second working part 111h have comparatively high strength due to work hardening.

FIG. 12 shows another example of a variable wall thickness steel pipe manufactured via the steps shown in FIGS. 10(a) to 10(d). A variable wall thickness steel pipe 121 shown in FIG. 12 is a variable wall thickness steel pipe manufactured by thrusting the plug 22 until the large-diameter base end portion 22b of the plug 22 reaches the one end portion 1a of the raw pipe 1, in the step shown in FIG. 10(d).

The variable wall thickness steel pipe 121 shown in FIG. 12 is configured to include a diameter-increasing portion 121c (1c) which is located on one end portion 121a side and is increased in diameter from the raw pipe 1, a diameter-increasing portion 121f (1c) which is located on the other end portion 121d (1d) side and is increased in diameter from the raw pipe 1, and a middle portion 121e (1e) which is located between the one end portion 121a and the other end portion 121d and is subjected to ironing. The middle portion 121e also includes a part subjected to working by the tapered portion 12c of the die 12 and the tapered portion 21c of the plug 21 at a boundary with respect to the diameter-increasing portion 121c, and a part subjected to working by the tapered portion 12e of the die 12 and the tapered portion 22c of the plug 22 at a boundary with respect to the diameter-increasing portion 121f. That is, the middle portion 121e includes a lock portion 121e1 (1g1) leading to the diameter-increasing portion 121c, and a lock portion 121e2 (1h1) leading to the diameter-increasing portion 121f.

In a hollow portion 121b of the variable wall thickness steel pipe 121, the entire inner diameter in its longitudinal direction is further increased than the inner diameter  $d_2$  of the raw pipe 1. In addition, the outer diameter of the variable wall thickness steel pipe 121 is further increased than the outer diameter  $d_1$  of the raw pipe 1 in the diameter-increasing portion 121c, lock portions 121e1 and 121e2 located at both ends of the middle portion 121e, and the diameter-increasing portion 121f. Moreover, a part excluding the lock portions 121e1 and 121e2 from the middle portion 121e remains unchanged as the outer diameter  $d_1$  of the raw pipe 1. Accordingly, the variable wall thickness steel pipe 121 has a comparatively great thickness in the diameter-increasing portion 121c and the diameter-increasing portion 121f and has a comparatively small thickness in the middle portion 121e.

In the variable wall thickness steel pipe 121 shown in FIG. 12, since a small working amount is applied to the diameter-increasing portion 121c and the diameter-increasing

ing portion **121f**, no work hardening has occurred in these part, or even if work hardening has occurred, it is very insignificant. Therefore, even in a case where post-working such as bending is performed with respect to the diameter-increasing portion **121c** or the diameter-increasing portion **121f**, annealing treatment or the like for softening work hardening becomes unnecessary.

In addition, since a comparatively large working amount is applied to the middle portion **121e**, the middle portion **121e** has comparatively high strength due to work hardening.

As described above, in the embodiment shown in FIGS. 10(a) to 11, the variable wall thickness steel pipe **111** is manufactured by using one die **12** and two plugs **21** and **22**. Therefore, the diameter-increasing portion **1c** (**121c**) and the diameter-increasing portion **1f** (**121f**) can be respectively provided on the one end portion **1a** side and the other end portion **1d** side of the raw pipe **1**. In addition, a region which remains unprocessed as the raw pipe **1** and regions subjected to ironing on both sides in the longitudinal direction can be provided in a region between the diameter-increasing portion **1c** and the diameter-increasing portion **1f** of the raw pipe **1**, so that it is possible to manufacture a variable wall thickness steel pipe in which the thickness varies in stages.

In the fifth embodiment described above, the variable wall thickness steel pipe **111** is manufactured by using the die **12** in a line symmetric shape having the one-dot chained line in FIGS. 10(a) to 10(d) as a symmetric axis. However, the die **12** may have a non-line symmetric shape, and the variable wall thickness steel pipe **111** may be manufactured by using two plugs of which the shapes are different from each other.

#### Sixth Embodiment

Next, a method of manufacturing a variable wall thickness steel pipe of a sixth embodiment will be described with reference to FIGS. 13(a) to 13(c). The method of manufacturing a variable wall thickness steel pipe of the present embodiment is configured to include a step similar to that of the first embodiment. In the present embodiment, the variable wall thickness steel pipe is manufactured by using a die **13** which is different from the die **11** used in the first embodiment. Since other configurations are similar to those of the first embodiment, a description will be omitted.

As shown in FIG. 13(a), the die **13** used in the present embodiment is configured to include a first hollow small-diameter portion **13a** and a second hollow small-diameter portion **13b** having an inner diameter corresponding to the outer diameter  $d_1$  of the raw pipe **1**, a thickly-formed portion **13e** being provided between the first hollow small-diameter portion **13a** and the second hollow small-diameter portion **13b**, a hollow large-diameter portion **13d** having an inner diameter  $d_3$  larger than the outer diameter  $d_1$  of the raw pipe **1**, and a tapered portion **13c** being provided between the first hollow small-diameter portion **13a** and the hollow large-diameter portion **13d**. The hollow large-diameter portion **13d**, the tapered portion **13c**, the first hollow small-diameter portion **13a**, the thickly-formed portion **13e**, and the second hollow small-diameter portion **13b** communicate with each other inside a die main body **13i**. In addition, the die **13** can be divided in the upward/downward direction on the sheet in FIG. 13(a).

The thickly-formed portion **13e** is configured to include a hollow intermediate-diameter portion **13f**, a tapered portion **13h** being provided between the hollow intermediate-diameter portion **13f** and the first hollow small-diameter portion **13a**, and a tapered portion **13g** being provided between the

hollow intermediate-diameter portion **13f** and the second hollow small-diameter portion **13b**. The inner diameter  $d_3$  of the hollow intermediate-diameter portion **13f** is set to be an inner diameter larger than the outer diameter  $d_1$  of the raw pipe **1** and to be an inner diameter smaller than the inner diameter of the hollow large-diameter portion **13d**. If the inner diameter  $d_3$  of the hollow intermediate-diameter portion **13f** is larger than the inner diameter of the hollow large-diameter portion **13d**, the raw pipe **1** is only subjected to pipe expanding in the hollow intermediate-diameter portion **13f** during the ironing step without being subjected to thinning. Therefore, the thickness of the raw pipe **1** in the thickly-formed portion **13e** remains unchanged as the original thickness of the raw pipe **1**.

Next, similar to the first embodiment, as shown in FIG. 13(b), the diameter-increasing step is performed. First, while the end portions of the die **13** and the raw pipe **1** on the sheet left side are in a fixed state, the small-diameter tip end portion **21a** and the large-diameter base end portion **21b** of the plug **21** are thrust into the one end portion **1a** of the raw pipe **1**. The plug **21** is thrust until the tapered portion **21c** reaches the position of the tapered portion **13c** of the die **13**. Accordingly, the diameter-increasing portion **1c** and the lock portion **1e1** are formed in the one end portion **1a** of the raw pipe **1**.

Next, as shown in FIG. 13(c), as the ironing step, in a state where the fixed state of the raw pipe **1** is released, whereas the fixed state of the die **13** is maintained, the plug **21** is further thrust toward the other end portion **1d** side of the raw pipe **1**. As the plug **21** is further thrust, the raw pipe **1** is pushed from the one end portion **1a** toward the other end portion **1d** side. However, since the lock portion **1e1** formed in the raw pipe **1** in the previous step remains locked in the tapered portion **13c** of the die **13**, the raw pipe **1** does not move. If the tapered portion **21c** and the large-diameter base end portion **21b** of the plug **21** are thrust to the position shown in FIG. 13(c), since the inner diameter  $d_3$  of the hollow intermediate-diameter portion **13f** of the die **13** is larger than the outer diameter  $d_1$  of the raw pipe **1**, the thickness portion of the raw pipe **1** flows into the thickly-formed portion **13e**. Accordingly, a thick portion **1j** is formed in the raw pipe **1**.

FIG. 14 shows a schematic cross-sectional view of a variable wall thickness steel pipe **141** manufactured via the steps shown in FIGS. 13(a) to 13(c). The variable wall thickness steel pipe **141** is configured to include a diameter-increasing portion **141c** (**1c**) which is located on one end portion **141a** (**1a**) side and is increased in diameter from the raw pipe **1**, a middle portion **141e** (**1e**) which is located between the one end portion **141a** and the other end portion **141d** (**1d**) and is subjected to ironing, and an unprocessed portion **141g** which is located on the other end portion **141d** side of the middle portion **141e** and remains unprocessed as the raw pipe **1**. The middle portion **141e** also includes a lock portion **141e1** (**1e1**) subjected to working by the tapered portion **13c** of the die **13** and the tapered portion **21c** of the plug **21** at a boundary with respect to the diameter-increasing portion **141c**, and a thick portion **141f** subjected to working by the thickly-formed portion **13e** of the die **13** and the tapered portion **21c** of the plug **21**.

A hollow portion **141b** of the variable wall thickness steel pipe **141** remains unchanged as the inner diameter  $d_2$  of the raw pipe **1** in the unprocessed portion **141g**, whereas a hollow portion **141b** of the variable wall thickness steel pipe **141** is further increased in diameter than the inner diameter  $d_2$  of the raw pipe **1** in the diameter-increasing portion **141c** and the middle portion **141e**. In addition, in the diameter-

increasing portion  $141c$ , a lock portion  $141e1$ , and the thick portion  $141f$ , the outer diameter of the variable wall thickness steel pipe  $141$  is further increased than the outer diameter  $d_1$  of the raw pipe  $1$ . In a part other than the thick portion  $141f$  and the lock portion  $141e1$  in the middle portion  $141e$ , and the unprocessed portion  $141g$ , the outer diameter  $d_1$  of the raw pipe  $1$  remains unchanged. Therefore, in a case of being seen in the longitudinal direction, the variable wall thickness steel pipe  $141$  has a constant inner diameter in the shape-increasing portion  $141g$  and a part of the middle portion  $141e$  excluding a portion thereof. Furthermore, the thick portion  $141f$  and the diameter-increasing portion  $141c$  have outer diameters different from each other.

In the variable wall thickness steel pipe  $141$  shown in FIG. 14, since a small working amount is applied to the diameter-increasing portion  $141c$  and the unprocessed portion  $141g$ , no work hardening has occurred in these parts, or even if work hardening has occurred, it is very insignificant. Therefore, the diameter-increasing portion  $141c$  and the unprocessed portion  $141g$  have low strength. Accordingly, even in a case where post-working such as bending is performed with respect to these parts, annealing treatment or the like for softening work hardening becomes unnecessary.

In addition, since a comparatively large working amount is applied to the middle portion  $141e$  of the variable wall thickness steel pipe  $141$ , the middle portion  $141e$  has comparatively high strength due to work hardening.

FIG. 15 shows another example of a variable wall thickness steel pipe manufactured via the steps shown in FIGS. 13(a) to 13(c). That is, in this example, in the step shown in FIG. 13(c), a variable wall thickness steel pipe  $151$  having a shape as shown in FIG. 15 is worked by thrusting the plug  $21$  until the large-diameter base end portion  $21b$  of the plug  $21$  reaches the other end portion  $1d$  of the raw pipe  $1$ .

The variable wall thickness steel pipe  $151$  shown in FIG. 15 is configured to include a diameter-increasing portion  $151c$  ( $1c$ ) which is located on one end portion  $151a$  ( $1a$ ) side and is increased in diameter from the raw pipe  $1$ , a middle portion  $151e$  ( $1e$ ) which is located between the one end portion  $151a$  and the other end portion  $151d$  ( $1d$ ) and is subjected to ironing, and the other end part  $151g$  which is located on the other end portion  $151d$  side of the middle portion  $151e$  and is subjected to ironing, similar to the middle portion  $151e$ . The middle portion  $151e$  includes a part subjected to working by the tapered portion  $13c$  of the die  $13$  and the tapered portion  $21c$  of the plug  $21$  at a boundary with respect to the diameter-increasing portion  $151c$ , and a thick portion  $151f$  subjected to working by the thickly-formed portion  $13e$  of the die  $13$  and the tapered portion  $21c$  of the plug  $21$ .

In a hollow portion  $151b$  of the variable wall thickness steel pipe  $151$ , the entire inner diameter in its longitudinal direction is further increased than the inner diameter  $d_2$  of the raw pipe  $1$ . In addition, the outer diameter of the variable wall thickness steel pipe  $151$  is further increased than the outer diameter  $d_1$  of the raw pipe  $1$  in the diameter-increasing portion  $151c$  and the thick portion  $151f$ . In the middle portion  $151e$  and the other end part  $151g$  other than the thick portion  $151f$ , the outer diameter  $d_1$  of the raw pipe  $1$  remains unchanged. Therefore, the variable wall thickness steel pipe  $151$  has an entirely constant inner diameter in the longitudinal direction and has a plurality of parts of which the outer diameters are different from each other.

In the variable wall thickness steel pipe  $151$  shown in FIG. 15, since a small working amount is applied to the diameter-increasing portion  $151c$ , no work hardening has occurred in this part, or even if work hardening has occurred,

it is very insignificant. Therefore, the diameter-increasing portion  $151c$  has comparatively low strength. Accordingly, even in a case where post-working such as bending is performed with respect to this part, annealing treatment or the like for softening work hardening becomes unnecessary.

In addition, since a comparatively large working amount is applied to the middle portion  $151e$  and the other end part  $151g$  of the variable wall thickness steel pipe  $151$ , the middle portion  $151e$  and the other end part  $151g$  have comparatively high strength due to work hardening.

As described above, in the embodiment shown in FIGS. 13(a) to 14, the variable wall thickness steel pipe  $141$  is manufactured by using the die  $13$  having the thickly-formed portion  $13e$  between the first hollow small-diameter portion  $13a$  and the second hollow small-diameter portion  $13b$ . Therefore, it is possible to manufacture the variable wall thickness steel pipe  $141$  having the thick portion  $1j$  ( $141f$ ) in the middle portion  $1e$  of the raw pipe  $1$  ( $141e$ ). In addition, it is possible to manufacture the variable wall thickness steel pipe  $141$  of which outer diameters are different from each other in the thick portion  $1j$  and the diameter-increasing portion  $1c$  ( $141c$ ).

In addition, in the variable wall thickness steel pipe  $141$ , since the working amount is comparatively small on the other end portion  $1d$  ( $141d$ ) side of the diameter-increasing portion  $1c$  and the middle portion  $1e$ , strength is low. Meanwhile, in the middle portion  $1e$  including the thick portion  $1j$ , since the working amount is comparatively large, strength is high.

#### Seventh Embodiment

Next, a method of manufacturing a variable wall thickness steel pipe of a seventh embodiment will be described with reference to FIGS. 16(a) to 16(c). The method of manufacturing a variable wall thickness steel pipe of the present embodiment is configured to include a step similar to that of the first embodiment. In the present embodiment, the variable wall thickness steel pipe is manufactured by using a plug  $161$  which is different from the plug  $21$  used in the first embodiment. Since other configurations are similar to those of the first embodiment, a description will be omitted.

As shown in FIG. 16(a), the plug  $161$  used in the present embodiment is configured to include a tapered tip end portion  $161b$  having a tip end portion  $161a$  having an outer diameter smaller than the inner diameter  $d_2$  of the raw pipe  $1$ , a large-diameter portion  $161c$  having a diameter  $d_5$  larger than the inner diameter  $d_2$  of the raw pipe  $1$  and smaller than the inner diameter  $d_1$  of the hollow small-diameter portion  $11a$  of the die  $11$ , and a small-diameter base end portion  $161e$  having a diameter  $d_4$  smaller than the diameter  $d_5$  of the large-diameter portion  $161c$ . A tapered portion  $161d$  is provided between the large-diameter portion  $161c$  and the small-diameter base end portion  $161e$ .

Similar to the first embodiment, as the diameter-increasing step shown in FIG. 16(b), while the sheet left sides of the die  $11$  and the raw pipe  $1$  are in a fixed state, the tapered tip end portion  $161b$  and the large-diameter portion  $161c$  of the plug  $161$  are thrust into the one end portion  $1a$  of the raw pipe  $1$ . The plug  $161$  is thrust until the tapered tip end portion  $161b$  reaches the position of the tapered portion  $11c$  of the die  $11$ . Accordingly, the diameter-increasing portion  $1c$  and the lock portion  $1e1$  are formed in the one end portion  $1a$  of the raw pipe  $1$ .

Next, as the ironing step shown in FIG. 16(c), in a state where the fixed state of the raw pipe  $1$  is released, whereas

the fixed state of the die 11 is maintained, the plug 161 is further thrust toward the other end portion 1d side of the raw pipe 1. As the plug 161 is further thrust, the raw pipe 1 is pushed from the one end portion 1a toward the other end portion 1d side. However, since the lock portion 1e1 formed in the raw pipe 1 in the previous step remains locked in the tapered portion 11c of the die 11, the raw pipe 1 does not move.

If the plug 161 is thrust as shown in FIG. 16(c), in the middle portion 1e of the raw pipe 1 in which the large-diameter portion 161c of the plug 161 is thrust, the original inner diameter  $d_2$  of the raw pipe 1 is increased to a size corresponding to the diameter  $d_5$  of the large-diameter portion 161c of the plug 161. At this time, since the diameter  $d_4$  of the small-diameter base end portion 161e succeeding the large-diameter portion 161c of the plug 161 is smaller than the diameter  $d_5$  of the large-diameter portion 161c, the small-diameter base end portion 161e does not come into contact with a part of the raw pipe 1 subjected to ironing. In this manner, in the ironing step, the plug 161 comes into contact with the raw pipe 1 in only the tapered tip end portion 161b and the large-diameter portion 161c. Accordingly, since a part of the plug 161 coming into contact with the raw pipe 1 is smaller than that of the first embodiment, frictional resistance between the raw pipe 1 and the plug 161 is reduced in the ironing step.

It is preferable that the difference  $(d_5 - d_4)$  between the diameter  $d_4$  of the small-diameter base end portion 161e of the plug 161 in FIG. 16(a) and the diameter  $d_5$  of the large-diameter portion 161c ranges as follows. That is, when the thickness of the raw pipe 1 is  $d_0$  and the thickness of the middle portion 1e after ironing is  $d$ , the difference between  $d_0$  and  $d$  ( $d_0 - d$ ) is defined as the amount  $t_d$  of thickness reduction. At this time, the amount  $t_d$  of thickness reduction and the difference  $(d_5 - d_4)$  between the diameter  $d_4$  of the small-diameter base end portion 161e and the diameter  $d_5$  of the large-diameter portion 161c is favorable to be  $2xt_d \geq (d_5 - d_4)$ . If the difference  $(d_5 - d_4)$  between the diameter  $d_5$  of the small-diameter base end portion 161e and the diameter  $d_4$  of the large-diameter portion 161c exceeds  $2xt_d$ , depending on the combination of the strength and the amount of thickness reduction of the material, the lock portion 1e1 of the raw pipe 1 can no longer be locked in the tapered portion 11c of the die 11 in the ironing step shown in FIG. 16(c).

A variable wall thickness steel pipe manufactured via the steps shown in FIGS. 16(a) to 16(c) has a shape similar to the variable wall thickness steel pipe 31 shown in FIG. 2. In addition, in the step shown in FIG. 16(c), the variable wall thickness steel pipe may be worked into a shape similar to that of the variable wall thickness steel pipe 41 shown in FIG. 3 by thrusting the plug 161 until the large-diameter portion 161c of the plug 161 reaches the other end portion 1d of the raw pipe 1.

As described above, in the present embodiment, as a variable wall thickness steel pipe is manufactured by using the plug 161 provided with the small-diameter base end portion 161e having a diameter smaller than the diameter of the large-diameter portion 161c, the ironing step can be performed without having the small-diameter base end portion 161e and a part of the raw pipe 1 subjected to ironing coming into contact with each other in the ironing step. That is, when the plug 161 is thrust, only the tapered tip end portion 161b and the large-diameter portion 161c come into slide contact with the inner surface of the raw pipe 1. In addition, when the plug 161 is pulled out, only the large-diameter portion 161c mainly comes into slide contact with the inner surface of the raw pipe 1. In this manner, when the

plug 161 is taken out and put in, since the small-diameter base end portion 161e does not come into slide contact with the inner surface of the raw pipe 1, compared to the first embodiment, frictional resistance between the raw pipe 1 and the plug 161 can be reduced when the plug 161 is taken out and put in the ironing step, and a force required for working can be prevented from being excessive.

#### Eighth Embodiment

A method of manufacturing a variable wall thickness steel pipe of an eighth embodiment has a step of performing drawing after ironing of the first to fourth embodiments and the sixth and seventh embodiments. In the present embodiment, as an example, the variable wall thickness steel pipe 61 manufactured via the step of the second embodiment is taken as an intermediate product 15, and drawing is performed with respect to the intermediate product 15.

First, a die 14 and the intermediate product 15 used in the present embodiment will be described with reference to FIGS. 17(a) and 17(b). The intermediate product 15 shown in FIG. 17(a) is the variable wall thickness steel pipe 61 manufactured via the step of the second embodiment. The intermediate product 15 is configured to include a diameter-increasing portion 15c which is located in one end portion 15a side and is increased in diameter from the raw pipe 1, a middle portion 15e which is located between the one end portion 15a and the other end portion 15d and is subjected to ironing, and an unprocessed portion 15f which is located on the other end portion 15d side of the middle portion 15e and remains unprocessed as the raw pipe 1. The middle portion 15e also includes a part subjected to working by the tapered portion 11c of the die 11 used in the second embodiment, and the tapered portions 51d and 51e of the plug 51 at each of boundaries with respect to the diameter-increasing portion 15c and the unprocessed portion 15f.

The die 14 shown in FIG. 17(a) is configured to include a hollow small-diameter portion 14b having an inner diameter corresponding to the outer diameters of the unprocessed portion 15f and the middle portion 15e of the intermediate product 15, and a tapered portion 14c leading to the hollow small-diameter portion 14b. The above-mentioned expression “the inner diameter corresponding to the outer diameters of the unprocessed portion 15f and the middle portion 15e” indicates a diameter size in which a gap size, to the extent that the hollow small-diameter portion 14b can be taken out and put in with respect to the inside and the outside, is added to the outer diameters of the unprocessed portion 15f and the middle portion 15e. In addition, the hollow small-diameter portion 14b and the tapered portion 14c communicate with each other inside a die main body 14e.

Since the outer diameters of the unprocessed portion 15f and the middle portion 15e of the intermediate product 15 are the same as the outer diameter  $d_1$  of the raw pipe 1, the inner diameter of the hollow small-diameter portion 14b corresponds to the outer diameter  $d_1$  of the raw pipe 1. The inner diameter of the tapered portion 14c becomes the largest diameter on one end portion 14a side of the die 14, and an inner diameter  $d_6$  at this position is set to a size larger than the outer diameter of the diameter-increasing portion 15c of the intermediate product 15.

Next, the method of manufacturing a variable wall thickness steel pipe according to the present embodiment will be described. First, the intermediate product 15 is manufac-

tured. Since the method of manufacturing the intermediate product **15** is similar to that of the second embodiment, a description will be omitted.

Next, as shown in FIGS. 17(a) and 17(b), in a state where the die **14** is fixed, the intermediate product **15** is inserted from the one end portion **14a** side toward the other end portion **14d** side of the die **14**. If a lock portion **15e1** of the intermediate product **15** reaches the position of the tapered portion **14c** of the die **14**, the diameter-increasing portion **15c** is locked in the tapered portion **14c**. However, the intermediate product **15** is further thrust to the other end portion **14d** side. Then, the lock portion **15e1** and the diameter-increasing portion **15c** are pressed by the tapered portion **14c**, so that the outer surfaces of the lock portion **15e1** and the diameter-increasing portion **15c** are pressurized, and drawing is performed with respect to the lock portion **15e1** and the diameter-increasing portion **15c** such that the outer diameters thereof are drawn.

If the intermediate product **15** is thrust to the position shown in FIG. 17(b), drawing is performed with respect to the lock portion **15e1** and the diameter-increasing portion **15c** in their entirety. Therefore, the entire outer diameter of the intermediate product **15** in the longitudinal direction becomes the same outer diameter as the inner diameter  $d_1$  of the hollow small-diameter portion **14b** of the die **14**.

FIG. 18 shows a schematic cross-sectional view of a variable wall thickness steel pipe **181** manufactured in accordance with the present embodiment. The variable wall thickness steel pipe **181** includes a diameter-reducing portion **181c** which is located on one end portion **181a** (**15a**) side and in which the diameter-increasing portion **15c** of the intermediate product **15** is subjected to drawing, and a part corresponding to the lock portion **15e1** which is subjected to drawing in the same manner. Meanwhile, other parts of the variable wall thickness steel pipe **181** are configured to include a middle portion **181e** (**15e**) which is not subjected to drawing and remains unchanged as the intermediate product **15**, and an unprocessed portion **181f** (**15f**) which is not subjected to drawing and remains unchanged as the intermediate product **15**.

In a hollow portion **181b** of the variable wall thickness steel pipe **181**, the entire outer diameter in its the longitudinal direction remains unchanged as the outer diameter of the raw pipe **1**. In addition, in the diameter-reducing portion **181c** and the unprocessed portion **181f**, the inner diameter of the variable wall thickness steel pipe **181** remains unchanged as the inner diameter  $d_2$  of the raw pipe **1**. In the middle portion **181e**, the inner diameter thereof is further increased than the inner diameter  $d_2$  of the raw pipe **1**. Therefore, the variable wall thickness steel pipe **181** has an entirely constant outer diameter in the longitudinal direction and has a plurality of regions of which the inner diameters are different from each other at positions in the longitudinal direction.

The variable wall thickness steel pipe **181** has a comparatively great thickness in the diameter-reducing portion **181c** and the unprocessed portion **181f** and has a comparatively small thickness in the middle portion **181e**.

In addition, in the variable wall thickness steel pipe **181**, since a small working amount is applied to the unprocessed portion **181f**, no work hardening has occurred in this part, or even if work hardening has occurred, it is very insignificant. Therefore, the unprocessed portion **181f** has comparatively low strength. Accordingly, even in a case where post-working such as bending is performed with respect to this part, annealing treatment or the like for softening work hardening becomes unnecessary.

In the present embodiment, as an example of the intermediate product **15**, the variable wall thickness steel pipe **61** manufactured in accordance with the second embodiment is employed. However, the present embodiment is not limited to only this example. For example, an intermediate product of the present embodiment may be the variable wall thickness steel pipe **31** which is manufactured in accordance with the first embodiment as shown in FIG. 2.

In addition, So that drawing is performed with respect to the entire outer surface of the intermediate product **15**, the inner diameter of the hollow small-diameter portion **14b** of the die **14** used in the present embodiment may be an inner diameter smaller than the outer diameter of the raw pipe **1**. In this case, if the inner diameter of the hollow small-diameter portion **14b** of the die **14** is excessively small with respect to the outer diameter of the raw pipe **1**, an opening drawing rate becomes excessively significant, so that there is concern that buckling may occur at the time of drawing. The opening drawing rate in this case will be described below.

Generally, as steel pipes for automobiles, steel pipes of which a ratio of the steel pipe thickness to the steel pipe outer diameter ( $t/D_0$ ,  $t$ : thickness of raw pipe and  $D_0$ : outer diameter of raw pipe) ranges from 0.001 to 0.15 are used. The inventors have minutely investigated the opening drawing rate in a case where drawing is performed with respect to a steel pipe having this size. As a result, it is ascertained that the opening drawing rate is favorably 0.4 or lower. Therefore, in a case where drawing is performed with respect to the entire outer surface of the intermediate product **15**, it is favorable that the inner diameter of the hollow small-diameter portion **14b** of the die **14** is set such that the opening drawing rate becomes 0.4 or lower. The opening drawing rate is expressed by the following Expression (1). The factor  $\kappa$  in the following Expression (1) indicates an opening drawing rate, the factor  $D_0$  indicates an outer diameter of a steel pipe before drawing, and the factor  $D$  indicates the outer diameter of the steel pipe after drawing.

$$K = (D_0 - D)/D_0 \quad (1)$$

As described above, in the present embodiment, it is possible to manufacture the variable wall thickness steel pipe **181** having an entirely constant outer diameter of the raw pipe **1** in the longitudinal direction and having a plurality of regions of which the inner diameters are different from each other. In this variable wall thickness steel pipe **181**, since a comparatively small working amount is applied to the unprocessed portion **181f**, strength in this region is comparatively low. In addition, since a comparatively large working amount is applied to the diameter-reducing portion **181c** and the middle portion **181e**, strength in these regions is comparatively high.

In addition, it is possible to manufacture a variable wall thickness steel pipe in which working is performed with respect to the entire region in the longitudinal direction, by performing drawing with respect to the entire outer surface of the intermediate product **15** in the longitudinal direction.

In addition, it is possible to manufacture a variable wall thickness steel pipe having an entirely constant outer diameter in the longitudinal direction and having a plurality of regions of which the inner diameters are different from each other. In this variable wall thickness steel pipe, since working is performed with respect to the entire region of the raw pipe **1** in the longitudinal direction, the strength of the entire region is higher than the original strength of the raw pipe **1**.

### Ninth Embodiment

A ninth embodiment will be described. A method of manufacturing a variable wall thickness steel pipe of the

present embodiment is configured to include a step similar to that of the first embodiment. In the present embodiment, the variable wall thickness steel pipe is manufactured by using a plug different from the plug 21 used in the first embodiment and the die 11 used in the first embodiment. Alternatively, the variable wall thickness steel pipe is manufactured by using a die different from the die 11 used in the first embodiment and the plug 21 used in the first embodiment. Since other configurations are similar to those of the first embodiment, a description will be omitted. Hereinafter, as an example of the ninth embodiment, the method of manufacturing a variable wall thickness steel pipe, in which a plug different from the plug 21 used in the first embodiment and the die 11 used in the first embodiment are used, will be described.

A plug 19 shown in FIG. 19 has a shape different from that of the plug 21 shown in FIG. 1(a). The shape of a cross section orthogonal to the longitudinal direction of the plug 19 is a quadrangular shape with rounded corners in its entirety in the longitudinal direction. In addition, the plug 19 is configured to include a small-sized tip end portion 19a, a large-sized base end portion 19b, and a tapered portion 19c provided between the small-sized tip end portion 19a and the large-sized base end portion 19b.

A diagonal length d7 of a cross section orthogonal to the longitudinal direction in the small-sized tip end portion 19a is a diameter corresponding to the inner diameter d<sub>2</sub> of the raw pipe 1. In a cross section orthogonal to the longitudinal direction in the large-sized base end portion 19b, a side length d8 of the quadrangular shape with rounded corners corresponds to the inner diameter d<sub>2</sub> of the raw pipe 1, and a diagonal length d9 is greater than the inner diameter d<sub>2</sub> of the raw pipe 1 and is smaller than the inner diameter d<sub>1</sub> of the hollow small-diameter portion 11a of the die 11.

If a variable wall thickness steel pipe is manufactured through a step similar to that of the first embodiment using the plug 19, a schematic view of a cross section orthogonal to the longitudinal direction in a middle portion subjected to ironing exhibits a shape as shown in FIG. 20(a). In the large-sized base end portion 19b of the plug 19, since the side length d8 corresponds to the inner diameter d<sub>2</sub> of the raw pipe 1 and the long diameter d9 is larger than the inner diameter d<sub>2</sub> of the raw pipe 1, a middle portion of a variable wall thickness steel pipe 20A manufactured by the plug 19 has an unprocessed portion 20a which remains unprocessed as the raw pipe 1, and a processed portion 20b, which has been subjected to ironing. Since the thickness of the unprocessed portion 20a remains unchanged as the raw pipe 1 and the working amount is small, strength thereof is comparatively low. Meanwhile, since the thickness of the processed portion 20b is comparatively small and the working amount is large, strength thereof is comparatively high. Therefore, in the middle portion subjected to ironing, the variable wall thickness steel pipe 20A manufactured in accordance with the present embodiment alternately has parts which are subjected to ironing and parts which remain unprocessed in the circumferential direction.

In the ninth embodiment described above, the variable wall thickness steel pipe 20A is manufactured through a step similar to the first embodiment using the plug 19 of which the shape of a cross section orthogonal to the longitudinal direction is a quadrangular shape with rounded corners, and the die 11. However, a plug having a different shape of a cross section orthogonal to the longitudinal direction may be used. However, it is favorable that a cross section orthogonal to the longitudinal direction of the plug has a rotationally symmetric shape. The reason is that in a case where a cross

section orthogonal to the longitudinal direction of the plug does not have a rotationally symmetric shape, the diameter-increasing portion cannot be sufficiently formed by performing pipe expanding and the raw pipe 1 cannot be locked in the tapered portion 11c of the die 11.

FIGS. 20(b) and 20(c) are views showing cross sections orthogonal to the longitudinal direction in middle portions of variable wall thickness steel pipes 20B and 20C manufactured by using different plugs of which cross sections orthogonal to the longitudinal direction in the eighth embodiment have a rotationally symmetric shape.

As described above, in the present embodiment, the variable wall thickness steel pipe may be manufactured by using a die different from the die 11 used in the first embodiment and the plug 21 used in the first embodiment. It is favorable that the die used in this case has a rotationally symmetric shape of a cross section orthogonal to the longitudinal direction of the die such that pipe expanding can be sufficiently performed. In addition, the outer shape of the raw pipe 1 has to be a shape corresponding to the die.

For example, if a variable wall thickness steel pipe 20D is manufactured by using a square-shaped steel pipe, a die having a shape corresponding to the square-shaped steel pipe, and the plug 21 similar to that of the first embodiment in a manner similar to that of the first embodiment, the shape of a cross section orthogonal to the longitudinal direction in the middle portion of the variable wall thickness steel pipe 20D becomes a shape as shown in FIG. 20(d).

FIG. 20(e) is a schematic cross-sectional view of the middle portion of a variable wall thickness steel pipe 20E in which the outer shape of a cross section of a raw pipe is an elliptic shape, and a die corresponding to the shape of and the raw pipe, and the plug 21 are used, and which is manufactured by a method similar to that of the first embodiment. In this case as well, the variable wall thickness steel pipe 20E alternately has parts which are subjected to ironing and parts which remain unprocessed in the circumferential direction.

As described above, according to the ninth embodiment, it is possible to manufacture the variable wall thickness steel pipe 20A alternately having parts which are subjected to ironing and parts which remain unprocessed in the circumferential direction, in a middle portion subjected to ironing. In addition, in the variable wall thickness steel pipe 20A, since the thickness of the parts subjected to ironing is small and the working amount is large, strength thereof is comparatively significant. Meanwhile, since the thickness of the parts which remain unprocessed is large and the working amount is small, strength thereof is comparatively small.

As described above, in the method of manufacturing a variable wall thickness steel pipe according to each of the embodiments of the present invention, the lock portion is provided by performing pipe expanding with respect to the raw pipe, and ironing is performed with respect to the middle portion on the other end side of the diameter-increasing portion of the raw pipe such that the inner diameter of the raw pipe is increased while the outer diameter is maintained, by thrusting the plug into the raw pipe while the lock portion is locked in the die. Therefore, the working amount with respect to the diameter-increasing portion can be reduced, so that heat treatment such as annealing can be made unnecessary when post-working such as bending is performed with respect to the diameter-increasing portion.

In addition, since ironing is performed by thrusting the plug into the raw pipe while the lock portion is locked in the

die, ironing can be carried out by only relatively moving the die and the plug without fixing the raw pipe itself at the time of ironing.

In addition, it is possible to form parts having a small thickness and comparatively high strength and parts having a large thickness and comparatively low strength in the longitudinal direction of the variable wall thickness steel pipe. Therefore, heat treatment such as annealing can be made unnecessary when post-working such as bending is performed with respect to a part having a large thickness and comparatively small strength.

Application examples of the variable wall thickness steel pipe in each of the embodiments of the present invention for automobile components include a frame member such as a cross-member, a suspension member, and a suspension arm; a collision countermeasure component such as a perimeter and a side impact bar; and a drive system pipe component such as a drive shaft.

In the frame member such as a cross-member, a suspension arm, and a suspension member, there are many cases where a large thickness is particularly required in attachment parts for other components. Therefore, by using the variable wall thickness steel pipe in each of the embodiments of the present invention it is possible to employ a light-weight structure in which only a required location is thickened. In addition, in these components, there are cases where pressing or bending is performed when performing post-working in which the thick portion is formed into a predetermined shape. In these cases, if a part to be subjected to working has a large thickness and low strength, it is easy to perform working. Therefore, it is possible to preferably use the variable wall thickness steel pipe in each of the embodiments of the present invention.

A side impact bar is a member which is installed inside a door panel and transmits collision energy at the time of a collision to both sides of a door, and it is desired that the side impact bar does not break at the time of a collision. Therefore, if a central portion is thickened by using the variable wall thickness steel pipe in each of the embodiments of the present invention, it is possible to realize a light-weight structure.

A perimeter is a frame member in the front part of a vehicle body, and the member becomes a load transmission path at the time of a frontal collision. The member can be further reduced in weight by causing a bending shape portion or the like which is likely to be bent at the time of a collision to be a thick portion. In addition, when a thick portion is bent, if the thick portion has low strength, it is easy to perform working. Therefore, it is possible to preferably use variable wall thickness steel pipe in each of the embodiments of the present invention.

In a drive shaft, there are cases where splining is performed with respect to variable wall thickness portions at pipe ends. If this part has a large thickness and low strength, it is easy to perform working. Therefore, it is possible to preferably use variable wall thickness steel pipe in each of the embodiments of the present invention.

Essentials of the above-described embodiments will be summarized below.

(1) For example, the method of manufacturing a variable wall thickness steel pipe according to the first embodiment described by using FIGS. 1(a) to 2 is a method of manufacturing a variable wall thickness steel pipe 31 with a hollow tubular (hollow cylindrical) raw pipe 1. The method includes locking the raw pipe 1 in a die 11 by thrusting a plug 21 into the raw pipe 1 from one end side (one end portion 1a), so as to expand (increase) an outer shape (outer

diameter) on the one end side, in a state where a raw pipe is disposed inside the die and movement of the raw pipe 1 in a longitudinal direction is restricted; and performing ironing in which an inner shape (inner diameter) of the raw pipe 1 is expanded while the outer shape (outer diameter) is maintained so that a thin portion 1e (31e) is formed by further thrusting the plug 21 toward the other end side (other end portion 1d) of the raw pipe 1 while the locked state of the raw pipe 1 is maintained, whereas the restriction on the raw pipe 1 is relaxed.

(2) Then, as shown in FIGS. 1(c) and 2, in the method of manufacturing a variable wall thickness steel pipe according to (1), in the performing ironing, an unprocessed portion 31f may remain on the other end side (other end portion 1d) of the raw pipe 1 by stopping thrusting the plug 21 in the middle.

(3) In addition, as shown in FIGS. 1(c) and 2, in the method of manufacturing a variable wall thickness steel pipe according to (1) or (2), a thickness reduction rate of the thin portion 1e (31e) in the performing ironing may be within a range from 10% to 90%.

(4) In addition, as shown in FIG. 1(c), in the method of manufacturing a variable wall thickness steel pipe according to any one of (1) to (3), the plug 21 used in the locking and the performing ironing may include a tip end portion (small-diameter tip end portion 21a) having an outer shape size (outer diameter size) smaller than an inner shape size (inner diameter size) of the raw pipe 1, a base end portion (large-diameter base end portion 21b) having an outer shape size (outer diameter size) larger than the inner shape size (inner diameter size) of the raw pipe 1 and smaller than an outer shape size (outer diameter size) of the raw pipe 1, and a tapered portion 21c being provided between the tip end portion (small-diameter tip end portion 21a) and the base end portion (large-diameter base end portion 21b) to be tapered from the base end portion (large-diameter base end portion 21b) toward the tip end portion (small-diameter tip end portion 21a).

(5) In addition, for example, as in the third embodiment described by using FIGS. 7(a) to 7(c), in the method of manufacturing a variable wall thickness steel pipe according to any one of (1) to (3), the plug 71 used in the locking and the performing ironing may include a base end portion 71b having an outer shape size (outer diameter size) larger than an inner shape size (inner diameter size) of the raw pipe 1 and smaller than an outer shape size (outer diameter size) of the raw pipe 1, and a tip end portion (tapered tip end portion 71c) leading to a tip end side of the base end portion 71b and being tapered as being separated from the base end portion 71b.

(6) In addition, for example, as in the seventh embodiment described by using FIGS. 16(a) to 16(c), in the method of manufacturing a variable wall thickness steel pipe according to (4) or (5), the base end portion may have a large-sized base end portion (large-diameter portion 161c) being disposed on the tip end portion side, and a small-sized base end portion (small-diameter base end portion 161e) having an outer shape size (outer diameter size) smaller than an outer shape size of the large-sized base end portion.

(7) For example, the method of manufacturing a variable wall thickness steel pipe according to the second embodiment described by using FIGS. 4(a) to 6 is a method of manufacturing a variable wall thickness steel pipe 61 with a hollow tubular (hollow cylindrical) raw pipe 1. The method includes locking the raw pipe 1 in a die 11 by thrusting a first plug (plug 21) into the raw pipe 1 from one end side (one end portion 1a), so as to expand (increase) an outer shape size

(outer diameter size) on the one end side (one end portion 1a), in a state where a raw pipe is disposed inside the die and movement of the raw pipe 1 in a longitudinal direction is restricted; pulling the first plug (plug 21) from the raw pipe 1; and performing ironing in which an inner shape (inner diameter) of the raw pipe 1 is expanded while an outer shape (outer diameter) of the raw pipe 1 is maintained so that a thin portion 1e (61e) is formed by thrusting a second plug (plug 51), which has an outer shape different from the outer shape of the first plug (plug 21), from the one end side (one end portion 1a) of the raw pipe 1 toward the other end side (other end portion 1d) while the locked state of the raw pipe 1 is maintained, whereas the restriction on the raw pipe 1 is relaxed.

(8) Then, as shown in FIGS. 5(a) and 5(b), in the method of manufacturing a variable wall thickness steel pipe according to (7), the second plug (plug 51) used in the performing ironing may include a small-sized tip end portion (small-diameter tip end portion 51a) smaller than an inner shape size (inner diameter size) of the raw pipe 1, an intermediate-sized portion (intermediate-diameter portion 51b) having an outer shape size (outer diameter size) larger than the inner shape size (inner diameter size) of the raw pipe 1, a large-sized portion (large-diameter base end portion 51c) having an outer shape size (outer diameter size) larger than the outer shape size (outer diameter size) of the intermediate-sized portion (intermediate-diameter portion 51b) and smaller than an outer shape size (outer diameter size) of the raw pipe 1, a first tapered portion (first tapered portion 51d) being provided between the small-sized tip end portion (small-diameter tip end portion 51a) and the intermediate-sized portion (intermediate-diameter portion 51b), and a second tapered portion (second tapered portion 51e) being provided between the intermediate-sized portion (intermediate-diameter portion 51b) and the large-sized portion (large-diameter base end portion 51c).

(9) In addition, as in the fourth embodiment described by using FIGS. 8(a) and 8(b), in the method of manufacturing a variable wall thickness steel pipe according to (7), the second plug (plug 81) used in the performing ironing may include a base end portion 81b having an outer shape size (outer diameter size) larger than the inner shape size (inner diameter size) of the raw pipe 1 and smaller than an outer shape size (outer diameter size) of the raw pipe 1, and a third tapered portion (tapered tip end portion 81c) being tapered from the base end portion 81b toward a tip end portion 81a.

(10) As in the first embodiment described by using FIGS. 1(a) to 1(c), in the method of manufacturing a variable wall thickness steel pipe according to any one of (1) to (9), the die 11 may include a hollow small-sized portion (hollow small-diameter portion 11a) having an inner shape size (inner diameter size) corresponding to the outer shape size (outer diameter size) of the raw pipe 1, a hollow large-sized portion (hollow large-diameter portion 11b) having an inner shape size (inner diameter size) larger than the outer shape size (outer diameter size) of the raw pipe 1, and a hollow tapered portion (tapered portion 11c) being provided between the hollow small-sized portion (hollow small-diameter portion 11a) and the hollow large-sized portion (hollow large-diameter portion 11b) and being tapered from the hollow large-sized portion (hollow large-diameter portion 11b) toward the hollow small-sized portion (hollow small-diameter portion 11a).

(11) As in the sixth embodiment described by using FIGS. 13(a) to 13(c), in the method of manufacturing a variable wall thickness steel pipe according to (10), the die 13 may further include a hollow intermediate-diameter portion

(thickly-formed portion 13e) being provided in a part of a hollow small-sized portion (hollow small-diameter portion 13a) in the longitudinal direction and having an inner shape size (inner diameter size) larger than the outer shape size (outer diameter size) of the raw pipe 1.

(12) As in the eighth embodiment described by using FIGS. 17(a) to 18, the method of manufacturing a variable wall thickness steel pipe according to any one of (1) to (11) may further include drawing the raw pipe 1 (intermediate product 15) after performing ironing.

(13) For example, the method of manufacturing a variable wall thickness steel pipe according to the fifth embodiment described by using FIGS. 10(a) to 11 is a method of manufacturing a variable wall thickness steel pipe 111 with a hollow tubular (hollow cylindrical) raw pipe 1. The method includes locking the raw pipe 1 in a die 12 by simultaneously or alternately thrusting plugs 21 and 22 into the raw pipe 1 respectively from one end side (one end portion 1a) and the other end side (other end portion 1d) of the raw pipe 1, so as to expand an outer shape (outer diameter) on the one end side (one end portion 1a) and an outer shape (outer diameter) on the other end side (other end portion 1d); pulling the plug 22 on the other end side (other end portion 1d) while the plug 21 is inserted on the one end side (one end portion 1a); performing first ironing in which an inner shape (inner diameter) of the raw pipe 1 is expanded while the outer shape (outer diameter) is maintained so that a first thin portion (middle portion 1g) is formed by further thrusting the plug 21, which is inserted on the one end side (one end portion 1a), toward the other end side (other end portion 1d) of the raw pipe 1 while the one end side (lock portion 1g1 on the one end portion 1a side) is locked in the die 12; inserting and pulling the plugs such that the plug 22 is inserted on the other end side (other end portion 1d), whereas the plug 21 on the one end side (one end portion 1a) is pulled out; and performing second ironing in which the inner shape (inner diameter) of the raw pipe 1 is expanded while the outer shape (outer diameter) is maintained so that a second thin portion (middle portion 1h) is formed by further thrusting the plug 22 on the other end side (other end portion 1d) toward the one end side (one end portion 1a) of the raw pipe 1 while the other end side (lock portion 1h1 on the other end portion 1d side) is locked in the die 12. In the locking, the raw pipe 1 freely moves in a longitudinal direction of the raw pipe 1 in a case where the plugs 21 and 22 are simultaneously thrust, and movement of the raw pipe 1 in a thrusting direction of the plugs 21 and 22 is restricted in a case where the plugs 21 and 22 are alternately thrust.

(14) According to the fifth embodiment shown in FIG. 11, the method of manufacturing a variable wall thickness steel pipe according to (13) may further include drawing the raw pipe 1 (variable wall thickness steel pipe 111) after performing second ironing.

(15) According to each of the embodiments, in the method of manufacturing a variable wall thickness steel pipe according to any one of (1) to (14), the raw pipe 1 may be a seamless steel pipe.

(16) For example, according to the first embodiment described by using FIG. 2, there is provided a variable wall thickness steel pipe 31 which employs the following configuration including an expanded portion (diameter-increasing portion 31c) that is provided on one side in a longitudinal direction and has a largest outer shape size (outer diameter size) in a case of being seen in a cross section perpendicular to the longitudinal direction, and a thin portion (middle portion 31e) that is provided on the other side of the expanded portion (diameter-increasing portion 31c) in a case

of being seen in the longitudinal direction and has a thickness smaller than the thickness of the expanded portion (diameter-increasing portion **31c**). In a case where an average value of hardness of the expanded portion (diameter-increasing portion **31c**) is  $H_1$  and an average value of hardness of the thin portion (middle portion **31e**) is  $H_2$ ,  $H_2 > H_1$  is satisfied.

(17) The variable wall thickness steel pipe **31** according to (16) may employ the following configuration further including a thick portion (unprocessed portion **31f**) that is disposed on the other side of the thin portion (middle portion **31e**) in a case of being seen in the longitudinal direction and has a thickness greater than the thickness of the thin portion (middle portion **31e**). In a case where an average value of hardness of the thick portion (unprocessed portion **31f**) is  $H_3$ ,  $H_2 > H_1 \geq H_3$  may be satisfied.

(18) For example, the variable wall thickness steel pipe **31** according to (17) may employ the following configuration in which the thin portion (middle portion **31e**) includes a straight pipe portion **31e2** having a smallest thickness in the thin portion (middle portion **31e**), a first tapered portion (lock portion **31e1**) being provided between the straight pipe portion **31e2** and the expanded portion (diameter-increasing portion **31c**) and having an outer shape (outer diameter) expanded toward the expanded portion (diameter-increasing portion **31c**), and a second tapered portion (tapered portion **31e3**) being provided between the straight pipe portion **31e2** and the thick portion (unprocessed portion **31f**) and having a thickness increasing toward the thick portion (unprocessed portion **31f**). In a case where an average value of hardness of the first tapered portion (lock portion **31e1**) is  $H_4$ , an average value of hardness of the straight pipe portion **31e2** is  $H_5$ , and an average value of hardness of the second tapered portion (tapered portion **31e3**) is  $H_6$ , both expressions  $H_5 > H_6 \geq H_3$  and  $H_5 > H_4 > H_1$  may be satisfied.

(19) According to the sixth embodiment described by using FIG. 14, in the variable wall thickness steel pipe **141** according to any one of (16) to (18), the thickness of the thin portion (middle portion **141e**) may be partially increased (thick portion **141f**) in a case of being seen in the longitudinal direction.

(20) According to the fifth embodiment described by using FIG. 11, in the variable wall thickness steel pipe **111** according to (16), combinations of the expanded portions (diameter-increasing portions **111c** and **111f**) and the thin portions (middle portions **111g** and **111h**) may be symmetrically provided at both ends in the longitudinal direction.

(21) The variable wall thickness steel pipe **111** according to (20) may employ the following configuration further including a thick portion (unprocessed portion **111i**) that is disposed between a pair of the thin portions (middle portions **111g** and **111h**) and has a thickness greater than the thickness of the thin portion (middle portions **111g** and **111h**). In a case where an average value of hardness of the thick portion (unprocessed portion **111i**) is  $H_7$ ,  $H_2 > H_1 \geq H_7$  may be satisfied.

(22) For example, according to the eighth embodiment described by using FIG. 18, there is provided a variable wall thickness steel pipe **181** which employs the following configuration including a thick portion (diameter-reducing portion **181c**) that is provided on one side in a longitudinal direction and has a greatest thickness in a case of being seen in a cross section perpendicular to the longitudinal direction, and a thin portion (middle portion **181e**) that is provided on the other side of the thick portion (diameter-reducing portion **181c**) and has a thickness smaller than the thickness of the thick portion (diameter-reducing portion **181c**). An outer

shape size in the longitudinal direction (outer diameter size) is constant. In a case where an average value of hardness of the thick portion (diameter-reducing portion **181c**) is  $H_8$  and an average value of hardness of the thin portion (middle portion **181e**) is  $H_9$ ,  $H_9 > H_8$  is satisfied.

(23) According to the ninth embodiment described by using FIG. 20(a), in the variable wall thickness steel pipe **20** according to any one of (16) to (22), in a case where the thin portion is seen in a circumferential direction of the thin portion in a cross section perpendicular to the longitudinal direction, the thin portion may have a rotationally symmetric shape in which regions (processed portion **20b**) having a relatively small thickness and relatively high hardness and regions (unprocessed portion **20a**) having a relatively great thickness and relatively low hardness alternate with each other in the circumferential direction.

(24) In the variable wall thickness steel pipe according to any one of (16) to (23), a seamless steel pipe may be used as a material.

## INDUSTRIAL APPLICABILITY

According to the present invention, it is possible to provide a method of manufacturing a variable wall thickness steel pipe, in which a working amount at the time of manufacturing is small and heat treatment such as annealing becomes unnecessary when post-working such as bending is performed, and a variable wall thickness steel pipe.

## BRIEF DESCRIPTION OF THE REFERENCE SYMBOLS

- 1 raw pipe
- 1a one end portion (one end side)
- 1d the other end portion (other end side)
- 1e, **31e**, **61e** thin portion
- 1g middle portion (first thin portion)
- 1g1 lock portion on one end portion side (one end side)
- 1h middle portion (second thin portion)
- 1h1 lock portion on the other end portion side (other end side)
- 11**, **12**, **13** die
- 11a hollow small-diameter portion (hollow small-sized portion)
- 11b hollow large-diameter portion (hollow large-sized portion)
- 11c tapered portion (hollow tapered portion)
- 13a hollow small-diameter portion (hollow small-sized portion)
- 13e thickly-formed portion (hollow intermediate-diameter portion)
- 20a unprocessed portion (region having large thickness and low hardness)
- 20b processed portion (region having small thickness and high hardness)
- 21 plug (first plug)
- 21a small-diameter tip end portion (tip end portion)
- 21b large-diameter base end portion (base end portion)
- 21c tapered portion
- 22**, **71** plug
- 31**, **61**, **111**, **141**, **181** variable wall thickness steel pipe
- 31c**, **41c**, **61c**, **91c**, **111c**, **111f**, **121c**, **141c**, **151c** diameter-increasing portion (expanded portion)
- 31e**, **111g**, **111h** middle portion (thin portion)
- 31e1** lock portion (first tapered portion)
- 31e2** straight pipe portion
- 31e3** tapered portion (second tapered portion)

39

- 31*f*, 111*i* unprocessed portion (unprocessed portion, thick portion)
- 51, 81 plug (second plug)
- 51*a* small-diameter tip end portion (small-sized tip end portion)
- 51*b* intermediate-diameter portion (intermediate-sized portion)
- 51*c* large-diameter base end portion (large-sized portion)
- 51*d* first tapered portion (first tapered portion)
- 71*b*, 81*b* base end portion
- 71*c* tapered tip end portion (tip end portion)
- 81*a* tip end portion
- 81*c* tapered tip end portion (third tapered portion)
- 141*e* middle portion (thin portion)
- 161*c* large-diameter portion (large-sized base end portion)
- 161*e* small-diameter base end portion (small-sized base end portion)
- 181*c* diameter-reducing portion (thick portion)
- 181*e* middle portion (thin portion)

The invention claimed is:

1. A method of manufacturing a variable wall thickness steel pipe with a hollow tubular raw pipe, the method comprising:

locking the raw pipe in a die by thrusting a plug into the raw pipe from an one end side, so as to expand an outer shape on the one end side, in a state where the raw pipe is disposed inside the die and movement of the raw pipe in a longitudinal direction is restricted; and

performing ironing in which an inner shape of the raw pipe is expanded while the outer shape is maintained so that a thin portion is formed by further thrusting the plug toward the other end side of the raw pipe while the locked state of the raw pipe is maintained, whereas the movement of a portion of the other end side of the raw pipe is unrestricted so that the portion of the other end side of the raw pipe is elongated in the longitudinal direction,

thereby obtaining the variable wall thickness steel pipe.

2. The method of manufacturing a variable wall thickness steel pipe according to claim 1, wherein in the performing ironing, an unprocessed portion remains on the other end side of the raw pipe by stopping thrusting the plug in the middle.

3. The method of manufacturing a variable wall thickness steel pipe according to claim 2, wherein a thickness reduction rate of the thin portion in the performing ironing is within a range from 10% to 90%.

4. The method of manufacturing a variable wall thickness steel pipe according to claim 2, wherein the plug used in the locking and the performing ironing includes,

a tip end portion having an outer shape size smaller than an inner shape size of the raw pipe,  
 a base end portion having an outer shape size larger than the inner shape size of the raw pipe and smaller than an outer shape size of the raw pipe, and  
 a tapered portion being provided between the tip end portion and the base end portion so as to be tapered from the base end portion toward the tip end portion.

5. The method of manufacturing a variable wall thickness steel pipe according to claim 1,

40

wherein a thickness reduction rate of the thin portion in the performing ironing is within a range from 10% to 90%.

6. The method of manufacturing a variable wall thickness steel pipe according to claim 5,

wherein the plug used in the locking and the performing ironing includes,

a tip end portion having an outer shape size smaller than an inner shape size of the raw pipe,  
 a base end portion having an outer shape size larger than the inner shape size of the raw pipe and smaller than an outer shape size of the raw pipe, and  
 a tapered portion being provided between the tip end portion and the base end portion so as to be tapered from the base end portion toward the tip end portion.

7. The method of manufacturing a variable wall thickness steel pipe according to claim 1,

wherein the plug used in the locking and the performing ironing includes,

a tip end portion having an outer shape size smaller than an inner shape size of the raw pipe,  
 a base end portion having an outer shape size larger than the inner shape size of the raw pipe and smaller than an outer shape size of the raw pipe, and  
 a tapered portion being provided between the tip end portion and the base end portion so as to be tapered from the base end portion toward the tip end portion.

8. The method of manufacturing a variable wall thickness steel pipe according to claim 7,

wherein the base end portion has a large-sized base end portion being disposed on the tip end portion side, and a small-sized base end portion having an outer shape size smaller than an outer shape size of the large-sized base end portion.

9. The method of manufacturing a variable wall thickness steel pipe according to claim 1,

wherein the die includes,

a hollow small-sized portion having an inner shape size corresponding to the outer shape size of the raw pipe,  
 a hollow large-sized portion having an inner shape size larger than the outer shape size of the raw pipe, and  
 a hollow tapered portion being provided between the hollow small-sized portion and the hollow large-sized portion and being tapered from the hollow large-sized portion toward the hollow small-sized portion.

10. The method of manufacturing a variable wall thickness steel pipe according to claim 9,

wherein the die further includes a hollow intermediate-diameter portion being provided in a part of the hollow small-sized portion in the longitudinal direction and having an inner shape size larger than the outer shape size of the raw pipe.

11. The method of manufacturing a variable wall thickness steel pipe according to claim 1, further comprising:

drawing the variable wall thickness steel pipe after performing ironing.

12. The method of manufacturing a variable wall thickness steel pipe according to claim 1,

wherein the raw pipe is a seamless steel pipe.

\* \* \* \* \*